



US005707943A

**United States Patent** [19]

Covitch

[11] **Patent Number:** **5,707,943**[45] **Date of Patent:** **Jan. 13, 1998**

[54] **MIXTURES OF ESTERIFIED CARBOXY-  
CONTAINING INTERPOLYMERS AND  
LUBRICANTS CONTAINING THEM**

[75] Inventor: **Michael J. Covitch, Cleveland Hts.,  
Ohio**

[73] Assignee: **The Lubrizol Corporation, Wickliffe,  
Ohio**

[21] Appl. No.: **767,399**

[22] Filed: **Dec. 16, 1996**

[51] Int. Cl.<sup>6</sup> ..... **C10M 145/10; C10M 149/00**

[52] U.S. Cl. ..... **508/466; 508/469; 508/472;  
525/217; 525/225; 525/227; 525/221; 525/329.5;  
525/330.3; 525/327.7**

[58] **Field of Search** ..... **508/466, 469,  
508/472; 525/217, 221, 225, 227, 327.7,  
329.5, 330.3**

[56] **References Cited**

**U.S. PATENT DOCUMENTS**

|           |         |           |            |
|-----------|---------|-----------|------------|
| 2,977,334 | 3/1961  | Zopf, Jr. | 252/51.5   |
| 2,992,987 | 7/1961  | Fields    | 151/56     |
| 3,085,994 | 4/1963  | Muskat    | 260/78.5   |
| 3,329,658 | 7/1967  | Fields    | 260/78.5   |
| 3,388,106 | 6/1968  | Muskat    | 260/78.5   |
| 3,392,155 | 7/1968  | Muskat    | 260/78.5   |
| 3,449,250 | 6/1969  | Fields    | 252/51.5   |
| 3,702,300 | 11/1972 | Coleman   | 252/51.5 A |
| 3,933,761 | 1/1976  | Coleman   | 260/78.5   |
| 3,956,149 | 5/1976  | Coleman   | 252/51.5 A |
| 3,959,159 | 5/1976  | Coleman   | 252/51.5 A |

|           |         |                |            |
|-----------|---------|----------------|------------|
| 4,088,589 | 5/1978  | Rossi et al.   | 252/56     |
| 4,180,637 | 12/1979 | Evani et al.   | 526/204    |
| 4,200,720 | 4/1980  | Evani et al.   | 526/233    |
| 4,284,414 | 8/1981  | Bryant         | 44/62      |
| 4,594,378 | 6/1986  | Tipton et al.  | 524/106    |
| 4,604,221 | 8/1986  | Bryant et al.  | 252/51.5 A |
| 4,654,050 | 3/1987  | Koch et al.    | 44/62      |
| 4,654,403 | 3/1987  | Tipton         | 525/194    |
| 4,734,446 | 3/1988  | Tipton         | 524/106    |
| 5,124,059 | 6/1992  | Koch et al.    | 252/56 R   |
| 5,157,088 | 10/1992 | Dishong et al. | 525/327.6  |
| 5,256,752 | 10/1993 | Dishong et al. | 526/329.5  |
| 5,283,235 | 2/1994  | Bush et al.    | 507/118    |
| 5,338,471 | 8/1994  | Lal            | 508/486    |
| 5,413,725 | 5/1995  | Lal et al.     | 508/487    |
| 5,641,734 | 6/1997  | Naegely        | 508/476    |

**OTHER PUBLICATIONS**

SAE Standard J300 (Dec. 1995).

H. Shaub, "A History of ASTM Accomplishments in Low Temperature Engine Oil Rheology" in Low Temperature Lubricant Rheology Measurement and Relevance to Engine Operation, R.B. Rhodes, ed., ASTM, Philadelphia, PA (1992), pp. 1-19 month unavailable.

*Primary Examiner*—Jacqueline V. Howard

*Attorney, Agent, or Firm*—Joseph P. Fischer; Frederick D. Hunter; James L. Cordek

[57] **ABSTRACT**

Mixtures of esterified carboxy-containing interpolymers and additive concentrates and lubricating oil compositions containing same. Residual acidity of the esterified interpolymers may be neutralized by reaction with an amine.

**26 Claims, No Drawings**

**MIXTURES OF ESTERIFIED CARBOXY-  
CONTAINING INTERPOLYMERS AND  
LUBRICANTS CONTAINING THEM**

**FIELD OF THE INVENTION**

This invention relates to compositions comprising mixtures of esterified carboxy-containing interpolymers and to lubricating compositions and additive concentrates containing such mixtures. More particularly, this invention relates to mixtures of esterified interpolymers derived from low molecular weight olefin or vinyl aromatic compounds and alpha, beta-unsaturated aliphatic acid, anhydride or ester thereof, such interpolymers being esterified with aliphatic alcohols and, optionally, neutralized with amino compounds having about one primary or secondary amino group. The resulting mixtures are particularly useful as pour point depressants.

**BACKGROUND OF THE INVENTION**

Ever since lubricating oils were prepared from crude oils, refiners have experienced difficulty with congealation of these products at low temperatures. Part of the difficulty arises from a natural stiffening at low temperatures of the hydrocarbons comprising the bulk of the oil. This type of congealation can be corrected quite easily by the use of a solvent such as kerosene to reduce the viscosity of the oil. The remainder of the difficulty arises from the crystallization at low temperatures of the paraffin wax present in almost all heavy mineral oil fractions. Upon crystallization, the paraffin wax tends to form interlocking networks which absorb oil and form a voluminous gel-like structure which restricts the flow or "pour" of the oil. Even though refining processes known as dewaxing have been developed to remove most of the paraffin from lubricating oil fractions, the small amount of wax remaining after dewaxing can cause serious problems. Even such small mounts of wax can raise by tens of degrees Fahrenheit the temperature at which an oil will flow freely as measured by a suitable "pour point" test. Since removal of the last traces of wax from oils is a difficult and costly matter, other answers have been sought by refiners.

Various pour point depressants have been developed and those to reach the commercial market have primarily been organic polymers, although some monomeric substances such as tetra (long chain alkyl) silicates, phenyl tristearoxy-silane, and pentaerythritol tetrastearate have been shown to be effective. Presently available commercial pour point depressants are believed to be represented by the following types of polymeric materials: polymethacrylates, for example, copolymers of various chain length alkyl methacrylates (see, for example, U.S. Pat. No. 2,655,479); polyacrylamides (see, for example, U.S. Pat. No. 2,387,501); Friedel-Crafts condensation products of chlorinated paraffin wax with naphthalene (see, for example, U.S. Pat. Nos. 1,815,022 and 2,015,748); Friedel-Crafts condensation products of chlorinated paraffin wax with phenol (see, for example, U.S. Pat. No. 2,191,498); and vinyl carboxylate, such as dialkyl fumarate copolymers (see, for example, U.S. Pat. Nos. 2,666,746; 2,721,877 and 2,721,878).

Esters of maleic anhydride/alpha-olefin copolymers have been suggested as pour point depressants. For example, U.S. Pat. No. 2,977,334 describes the use of copolymers of maleic anhydride and ethylene which are esterified with low or high molecular weight alcohols and/or amidized with an amine. These resins are described as being useful as pour point modifiers, gelling agents, thickeners, viscosity improvers, etc., for mineral and synthetic oils including

functional fluids and lubricating oils. U.S. Pat. No. 2,992,987 describes a class of lubricant additives useful as pour point depressants which are ethylene-maleic anhydride copolymers esterified to 80% or more, preferably 90-100%, with a mixture of straight-chain saturated hydrocarbon alcohols having from 8 to 24 carbon atoms. The unesterified carboxylic groups can be left unreacted or can be reacted with such materials as ethylene or propylene oxide alcohol esters, or lower-dialkyl-amino-lower-alkylene-amines. U.S. Pat. Nos. 3,329,658 and 3,449,250 describe copolymers of maleic anhydride and alpha-olefins such as ethylene, propylene, isobutylene or vinyl aromatic compounds such as styrene as being useful dispersancy and detergency additives for oils, as well as pour point depressants and viscosity index improvers. The copolymer is esterified to about 30 to about 95% with aliphatic alcohols or mixtures of alcohols having from 10 to 20 carbon atoms, and the remaining carboxyl groups are reacted with an amine of the following formula:



where  $R_1$  and  $R_2$  are selected from the group consisting of aliphatic hydrocarbon radicals having from 1 to 4 carbon atoms and the cyclohexyl radical,  $R_3$  is an aliphatic hydrocarbon radical having from 2 to 4 carbon atoms, and  $R_4$  is selected from the class consisting of hydrocarbon atom and aliphatic hydrocarbon radicals having from 1 to 4 carbon atoms.

U.S. Pat. Nos. 3,702,300 and 3,933,761 describe carboxy-containing interpolymers in which some of the carboxy radicals are esterified and the remaining carboxy radicals are neutralized by reaction with a polyamino compound having one primary or secondary amino group and at least one mono-functional amino group, and indicate that such interpolymers are useful as viscosity index improving and anti-sludge agents in lubricating compositions and fuels. The patentee indicates that it is critical that the mixed esters described in these patents include both relatively high molecular weight carboxylic ester groups having at least eight aliphatic carbon atoms in the ester radical and relatively low molecular weight carboxylic ester groups having no more than seven aliphatic carbon atoms in the ester radical.

U.S. Pat. No. 4,604,221 relates to interpolymers similar to those described in the aforementioned '300 and '761 patents, except the ester groups contain at least 8 carbon atoms in the ester radical.

U.S. Pat. No. 5,124,059 describes esters of similar interpolymers characterized by the presence within its polymeric structure of the following groups which are derived from carboxy groups of said interpolymer:

- (A) at least one carboxylic ester group having at least 8 aliphatic carbon atoms in the ester group;
- (B) at least one carboxylic ester group having an ester group of the formula



wherein  $R$  is a hydrocarbyl group of about 1 to about 50 carbon atoms,  $R'$  is a hydrocarbyl group of about 1 to about 50 carbon atoms,  $y$  is a number in the range of zero to about 50 and  $z$  is a number in the range of zero to about 50 with the proviso that both  $y$  and  $z$  cannot be zero; and optionally

(C) at least one carboxylic ester group having no more than 7 aliphatic carbon atoms in the ester group.

U.S. Pat. No. 3,956,149 issued to Coleman relates to a lubricant or fuel composition containing a nitrogen-containing ester of a carboxy-containing interpolymer.

U.S. Pat. No. 3,959,159 issued to Coleman relates to lubricating compositions containing a nitrogen-containing mixed ester of a carboxy-containing interpolymer.

U.S. Pat. No. 4,284,414 issued to Bryant relates to a crude oil composition containing mixed alkyl esters of a carboxy-containing interpolymer.

U.S. Pat. No. 4,180,637 issued to Evani et al. relates to a process for preparing a low molecular weight carboxy-containing copolymer.

U.S. Pat. No. 4,200,720 issued to Evani et al. relates to a process for preparing a low molecular weight carboxy-containing interpolymer.

U.S. Pat. No. 3,085,994 issued to Muskat relates to a carboxy-containing interpolymer.

U.S. Pat. No. 3,388,106 issued to Muskat relates to a process for making a carboxy-containing interpolymer.

U.S. Pat. No. 3,392,155 issued to Muskat relates to a polyoxy alkylene glycol ester of a carboxy-containing interpolymer.

U.S. Pat. No. 5,157,088 relates to nitrogen-containing esters of carboxy-containing interpolymers having relatively 25 low inherent viscosity.

U.S. Pat. No. 4,088,589 relates to lubricating oils blended from petroleum distillates and, if desired, a bright stock containing waxy or wax-like components and modified by the presence of copolymeric ethylene-higher alpha-olefins viscosity index improving agents, having their low temperature performance improved when said copolymer contains a minor weight proportion of ethylene by the addition of from 0.15 to 1%, based on the total weight of said lubricating oil 30 composition of a combination of pour point depressants comprising: (a) from about 0.05 to about 0.75 wt. % of an oil-soluble condensation product of a chlorinated wax of from 10 to 50 carbon atoms and a mono- or dinuclear aromatic compound; and (b) from 0.05 to 0.75 wt. % of an oil soluble polymer of  $C_{10-18}$  alkyl acrylate and/or an interpolymer of a vinyl alcohol ester of a  $C_2$  to  $C_{18}$  alkanoic acid and di-( $C_4-C_{18}$  alkyl) fumarate.

The Society of Automotive Engineers (SAE) has issued a standard, J-300 (December 1995), which defines limits for classification of engine lubricating oils in rheological terms. This standard contains limits for various engine oil viscosity 45 grades. Also included in the standard are discussions of low temperature and of high temperature test methods.

A review of developments in low temperature performance is presented by Schaub, "A History of ASTM Accomplishments in Low Temperature Engine Oil Rheology" in "Low Temperature Lubricant Rheology Measurement and Relevance to Engine Operation", R. B. Rhodes, ed., ASTM, Philadelphia, Pa. (1992), pp 1-19.

Although many pour point depressants have been suggested and many are available in the market, concerted efforts are constantly being made to find new pour point depressants which are more economical and more effective than the depressants heretofore known in the art. In particular, a great deal of interest exists in pour point depressants which are capable of imparting other desirable properties to the lubricating compositions to which they are added in addition to pour point depressant properties.

#### SUMMARY OF THE INVENTION

Mixtures of esterified carboxy-containing interpolymers are provided in accordance with the present invention which

when added to lubricant compositions provide such lubricant compositions with superior low temperature properties as well as other desirable properties including viscosity index improvement. These esters, particularly the nitrogen-containing esters, also enhance the dispersion of other additives as well as contaminants (e.g., dirt, water, metallic particles, etc.) in the lubricating compositions to which they are added. These esters also enhance the flow characteristics of additive concentrates to which they are added.

10 Broadly stated, the present invention contemplates the provision of a composition comprising a mixture of esterified carboxy-containing interpolymers, said interpolymers having a reduced specific viscosity (abbreviated as RSV) of from about 0.05 to about 2 and being derived from at least 15 two monomers comprising (i) a  $C_{2-30}$  aliphatic olefin or vinyl aromatic compound and (ii) an alpha, beta-unsaturated acylating agent, preferably an aliphatic acid, anhydride or esters thereof. Nitrogen-containing esters are substantially free of titratable acidity. The mixture of esterified interpolymers is characterized by the presence therein of at least two members of the group consisting of

(I) an ester which within its polymeric structure consists essentially of

(A) pendant carboxylic ester groups which are derived from the carboxy groups of said interpolymers, said carboxylic ester groups containing at least 8 carbon atoms;

(II) an ester which is a mixed ester of said carboxy-containing interpolymers and being characterized by the presence within its polymeric structure of at least one of each of two ester groups:

(B) relatively high molecular weight pendant carboxylic ester groups containing at least eight aliphatic carbon atoms, and

(C) relatively low molecular weight pendant carboxylic ester groups containing no more than seven aliphatic carbon atoms, wherein the molar ratio of (B):(C) is (70-95):(5-30);

(III) an ester which is a nitrogen-containing ester, and which within its polymeric structure consists essentially of

(A) pendant carboxylic ester groups which are derived from the carboxy groups of said interpolymers, said carboxylic ester groups containing at least 8 carbon atoms, and

(D) pendant carbonyl-amino groups derived from amino compounds having an average of from 1 to about 1.1 primary or secondary amino group, wherein the molar ratio of carboxy groups of said interpolymer esterified to provide (A) to carboxy groups of said interpolymer neutralized to provide (D) is in the range of from about 85:15 to about 99:1; and

(IV) an ester which is a nitrogen containing ester, which is a mixed ester of said carboxy-containing interpolymers and being characterized by the presence within its polymeric structure of at least one of each of three groups:

(B) relatively high molecular weight pendant carboxylic ester groups containing at least eight aliphatic carbon atoms,

(C) relatively low molecular weight carboxylic ester groups containing no more than seven aliphatic carbon atoms, and

(E) carbonyl-amino groups derived from an amino compound having an average of from 1 to about 1.1

primary or secondary amino group, wherein the molar ratio of (B):(C):(E) is (60-94):(5-30):(1-15); and wherein the at least two members include at least one ester having the carboxylic ester group (A) and at least one ester having the carboxylic ester groups (B) and (C).

Lubricant compositions and additive concentrates comprising the foregoing mixture of esterified interpolymers are also provided in accordance with the present invention. Further, the present invention contemplates the provision of a process for making the mixture of esterified carboxy-containing interpolymers.

#### DETAILED DESCRIPTION OF THE PREFERRED EMBODIMENTS

As used herein, the terms "hydrocarbon", "hydrocarbyl" or "hydrocarbon based" mean that the group being described has predominantly hydrocarbon character within the context of this invention. These include groups that are purely hydrocarbon in nature, that is, they contain only carbon and hydrogen. They may also include groups containing substituents or atoms which do not alter the predominantly hydrocarbon character of the group. Such substituents may include halo-, alkoxy-, nitro-, etc. These groups also may contain hetero atoms. Suitable hetero atoms will be apparent to those skilled in the art and include, for example, sulfur, nitrogen and oxygen. Therefore, while remaining predominantly hydrocarbon in character within the context of this invention, these groups may contain atoms other than carbon present in a chain or ring otherwise composed of carbon atoms.

In general, no more than about three non-hydrocarbon substituents or hetero atoms, and preferably no more than one, will be present for every 10 carbon atoms in the hydrocarbon or hydrocarbon based groups. Most preferably, the groups are purely hydrocarbon in nature, that is, they are essentially free of atoms other than carbon and hydrogen.

Throughout the specification and claims the expression oil soluble or dispersible is used. By oil soluble or dispersible is meant that an amount needed to provide the desired level of activity or performance can be incorporated by being dissolved, dispersed or suspended in an oil of lubricating viscosity. Usually, this means that at least about 0.001% by weight of the material can be incorporated in a lubricating oil composition. For a further discussion of the terms oil soluble and dispersible, particularly "stably dispersible", see U.S. Pat. No. 4,320,019 which is expressly incorporated herein by reference for relevant teachings in this regard.

In the context of this invention the term "interpolymer" means a polymer derived from two or more different monomers.

As used in the specification and claims, the term carboxy-containing refers to polymers which are prepared using a carboxy-containing monomer. The carboxy-containing monomer is polymerized with other monomers to form the carboxy-containing interpolymer. Since the carboxy-containing monomer is incorporated into the polymer backbone, the carboxy groups extend from the polymer backbone, e.g., the carboxy groups are directly attached to the polymer backbone.

As described above, the invention relates to compositions containing a mixture of esterified carboxy-containing interpolymers. The mixture may comprise amounts ranging from about 1-99% by weight, preferably from about 5 to about 95% by weight, and more often from about 15 to about 85% by weight of esters having carboxylic ester group (A), and

from about 99-1% by weight, preferably from about 95 to about 5% by weight, and more often from about 85 to about 15% by weight of esters having carboxylic ester groups (B) and (C).

In reference to the size of the ester groups, it is pointed out that an ester group is represented by the formula



and that the number of carbon atoms in an ester group is thus the combined total of the carbon atom of the carbonyl group and the carbon atoms of the (OR) group.

An essential element of the present invention is the presence of the mixture of esterified interpolymers. The mixture is critical to the improved low temperature properties.

An optional element of the present invention is the presence of an amino group derived from amino compounds, and particularly those having an average of from 1 to about 1.1 primary or secondary amino groups. In one embodiment the amino compound is a polyamino compound having at least one mono-functional amino group. Such amino groups, when present in the esters of the present invention in the proportion stated above, enhance the dispersability of such esters in lubricant compositions and additives for lubricant compositions.

When the mixture contains a nitrogen-containing ester, an essential element is the extent of esterification in relation to the extent of neutralization of the unesterified carboxy groups of the carboxy-containing interpolymer through the conversion thereof to amino-containing groups. The molar ratio of the carboxy groups of said interpolymer that are esterified to the carboxy groups neutralized through the conversion thereof to amino-containing groups is generally in the range of about 85:15 to about 99:1. A preferred ratio is 95:5. It should be noted that the linkage described as the carbonyl-amino group may be salt, imide, amide, amidine and inasmuch as any such linkage is contemplated within the present invention, the term "carbonyl amino" is thought to be a convenient, generic expression useful for the purpose of defining the inventive concept. In a particularly advantageous embodiment of the invention such linkage is imide or predominantly imide.

Still another important element of the present invention is the molecular weight of the carboxy-containing interpolymer before esterification. Whenever reference is made in this application to RSV or reduced specific viscosity, the reference is to the interpolymer before it is esterified. For convenience, the molecular weight is expressed in terms of the "reduced specific viscosity" of the interpolymer which is a widely recognized means of expressing the molecular size of a polymeric substance. As used herein, the reduced specific viscosity (abbreviated RSV) is the value obtained in accordance with the formula

$$\text{RSV} = \frac{\text{Relative Viscosity} - 1}{\text{Concentration}}$$

wherein the relative viscosity is determined by measuring, by means of a dilution viscometer, the viscosity of a solution of one gram of the interpolymer in 100 ml. of acetone and the viscosity of acetone at  $30^\circ \pm 0.02^\circ \text{ C}$ . For purpose of computation by the above formula, the concentration is adjusted to 0.4 gram of the interpolymer per 100 ml. of acetone. A more detailed discussion of the reduced specific viscosity, also known as the reduced viscosity, as well as its relationship to the average molecular weight of an interpolymer, appears in Paul J. Flory, *Principles of Polymer*

*Chemistry*, (1953 Edition) pages 308 et seq; Mark, Bikales, Overberger and Menges, Eds., *Encyclopedia of Polymer Science and Engineering*, 2nd ed., Wiley Interscience (1988), V. 14, pp 463-465; and F. W. Billmeyer, *Textbook Of Polymer Science*, Wiley Publishing (1962), pp 79-85.

### The Interpolymer

The carboxy-containing interpolymers useful in preparing the esters useful in the invention are copolymers, terpolymers, and other interpolymers of (i) at least one aliphatic olefin monomer or vinyl aromatic monomer, and (ii) at least one alpha, beta-unsaturated carboxylic acylating agent, typically a carboxylic acid or derivative thereof. The derivatives of the carboxylic acid are derivatives which are polymerizable with the olefin monomers or vinyl aromatic monomers (i), and as such may be the esters, especially lower alkyl esters, e.g., those containing from 1 to 7 carbon atoms, especially 1-2 carbon atoms, halides and anhydrides of the acids. The molar ratio of (i) to (ii) ranges from about 1:2 to about 3:1, preferably about 1:1. The carboxy-containing interpolymer is prepared by polymerizing an aliphatic olefin or vinyl aromatic monomer with the alpha, beta-unsaturated carboxylic acid or derivative thereof.

Mixtures of two or more compatible (i.e., nonreactive to one another) interpolymers which are separately prepared are contemplated herein for use in the esterification reaction, if each has a RSV as above described. Thus, as used herein, and in the appended claims, the terminology "interpolymer" refers to either one separately prepared interpolymer or a mixture of two or more of such interpolymers. A separately prepared interpolymer is one in which the reactants and/or reaction conditions are different from the preparation of another interpolymer.

While interpolymers having RSV from about 0.05 to about 2 are contemplated in the present invention, the preferred interpolymers are those having RSV of from about 0.08, often from 0.2 or 0.35 to about 1.2, often to 0.8 or 1. In another embodiment, the RSV ranges from about 0.05 to about 0.9, in still another embodiment, from about 0.08 to about 0.9. Interpolymers having RSV of from about 0.35 to about 0.5 or from about 0.65 to about 0.75 are particularly useful.

### Aliphatic Olefins

Suitable aliphatic olefin monomers that are useful in the preparation of the interpolymers of the invention are mono-olefins of about 2 to about 30 carbon atoms. Included in this group are internal olefins (i.e., wherein the olefinic unsaturation is not in the "1" or alpha position) and mono-1-olefins or alpha-olefins. Alpha olefins are preferred. Exemplary olefins include ethylene, propylene, 1-butene, isobutene, 1-pentene, 2-methyl-1-butene, 3-methyl-1-butene, 1-hexene, 1-heptene, 1-octene, 1-dodecene, 1-tridecene, 1-tetradecene, 1-pentadecene, 1-hexadecene, 1-heptadecene, 1-octadecene, 1-nonadecene, 1-eicosene, 1-heneicosene, 1-docosene, 1-tetracosene, 1-pentacosene, 1-hexacosene, 1-octacosene, 1-nonacosene, etc. Commercially available alpha-olefin can also be used. Exemplary alpha-olefin mixtures include C<sub>15-18</sub> alpha-olefins, C<sub>12-16</sub> alpha-olefins, C<sub>14-16</sub> alpha-olefins, C<sub>14-18</sub> alpha-olefins, C<sub>16-18</sub> alpha-olefins, C<sub>16-20</sub> alpha-olefins, C<sub>22-28</sub> alpha-olefins, etc. Additionally, C<sub>30+</sub> alpha-olefin fractions such as those available from Conoco, Inc. can be used. Preferred olefin monomers include ethylene, propylene and 1-butene.

The mono-olefins can be derived from the cracking of paraffin wax. The wax cracking process yields both even and

odd number C<sub>6-20</sub> liquid olefins of which 85 to 90% are straight chain 1 olefins. The balance of the cracked wax olefins is made up of internal olefins, branched olefins, diolefins, aromatics and impurities. Distillation of the C<sub>6-20</sub> liquid olefins obtained from the wax cracking process yields fractions (e.g., C<sub>15-18</sub> alpha-olefins) which are useful in preparing the interpolymers of this invention.

Other mono-olefins can be derived from the ethylene chain growth process. This process yields even numbered straight chain 1-olefins from a controlled Ziegler polymerization.

Other methods for preparing the mono-olefins of this invention include chlorination-dehydrochlorination of paraffin and catalytic dehydrogenation of paraffins.

The above procedures for the preparation of mono-olefins are well known to those of ordinary skill in the art and are described in detail under the heading "Olefins" in the Encyclopedia of Chemical Technology, Second Edition, Kirk and Othmer, Supplement, pages 632-657, Interscience Publishers, Div. of John Wiley and Son, 1971, which is hereby incorporated by reference for its relevant disclosures pertaining to methods for preparing mono-olefins.

### Vinyl Aromatic Monomers

Suitable vinyl aromatic monomers which can be polymerized with the alpha, beta-unsaturated acylating agents include styrene and the substituted styrenes although other vinyl aromatic monomers can also be used. The substituted styrenes include styrenes that have halo-, amino-, alkoxy-, carboxy-, hydroxy-, sulfonyl-, hydrocarbyl- wherein the hydrocarbyl group has from 1 to about 12 carbon atoms and other substituents. Exemplary of the hydrocarbyl-substituted styrenes are alpha-methylstyrene, para-tert-butylstyrene, alpha-ethylstyrene, and para-lower alkoxy styrene. Mixtures of two or more vinyl aromatic monomers can be used. Styrene is preferred.

### Alpha, Beta-Unsaturated Acylating Agent

Suitable alpha, beta-unsaturated acylating agents useful in the preparation of the interpolymers are represented by carboxylic acids, anhydrides, halides, or lower alkyl esters thereof. These include mono-carboxylic acids (e.g., acrylic acid, methacrylic acid, etc. or lower alkyl esters thereof, as well as dicarboxylic acids, anhydrides or lower alkyl esters thereof wherein a carbon-to-carbon double bond is in an alpha, beta- position to at least one of the carboxy functions (e.g., itaconic acid, anhydride or lower esters thereof,  $\alpha$ -methylene glutaric acid or esters thereof,) and preferably in an alpha, beta-position to both of the carboxy functions of the alpha, beta-dicarboxylic acid, anhydride or the lower alkyl ester thereof (e.g., maleic acid or anhydride, fumaric acid, or lower alkyl esters thereof). Normally, the carboxy functions of these compounds will be separated by up to about 4 carbon atoms, preferably about 2 carbon atoms.

A class of preferred alpha, beta-unsaturated dicarboxylic acid, anhydrides or the lower alkyl esters thereof, includes those compounds corresponding to the formulae:



9



(II)

10

acrylonitrile, vinyl pyrrolidinone, vinyl pyridine, vinyl ethers, and vinyl carboxylates. In one embodiment, the additional comonomers are vinyl ethers or vinyl carboxylates.

- 5 Vinyl ethers are represented by the formula  $R_1-CH=CH-OR_2$  wherein each  $R_1$  is hydrogen or a hydrocarbyl group having 1 to about 30, or to about 24, or to about 12 carbon atoms and  $R_2$  is a hydrocarbyl group having 1 to about 30 carbon atoms, or to about 24, or to about 12. Examples of vinyl ethers include vinyl methylether, vinyl propylether, vinyl 2-ethylhexylether and the like.

10 The vinyl ester of a carboxylic acid may be represented by the formula  $R_3CH=CH-O(O)CR_4$  wherein  $R_3$  is a hydrogen or hydrocarbyl group having from 1 to about 30, or to 15 12 carbon atoms, or just hydrogen, and  $R_4$  is a hydrocarbyl group having 1 to about 30, or to about 12, or to about 8. Examples of vinyl esters include vinyl acetate, vinyl 2-ethylhexanoate, vinyl butanoate, vinyl crotonate. Vinyl 20 carboxylates include vinyl acetate, vinyl butanoate, etc.

15 The molecular weight (i.e., RSV) of such interpolymers can be adjusted to the range required in this invention, if necessary, according to conventional techniques, e.g., control of the reaction conditions.

20 The following examples serve to illustrate the preparation of the interpolymers used in this invention and are not intended as limiting thereof. Unless otherwise indicated, in the following examples as well as throughout the specification and in the appended claims, all parts and percentages 25 are by weight and all temperatures in degrees Celsius. RSV values are for diluent-free polymers in deciliters per gram @ 30 30° C. Benzoyl peroxide is nominally 70% in  $H_2O$ . Peradox 16 is nominally 98-99% assay bis(4-t-butylcyclohexyl) 35 peroxydicarbonate.

#### EXAMPLE 1

A styrene-maleic interpolymer is obtained by reacting 16.3 parts styrene and 11.9 parts of maleic anhydride in 40 272.7 parts of a benzene-toluene solvent mixture (weight ratio of benzene:toluene being 66.5:33.5) at 86° C. in a nitrogen atmosphere for 8 hours with 0.42 part of benzoyl 45 peroxide catalyst. The resulting product is a thick slurry of the interpolymer in the solvent mixture. To the slurry there is added 141 parts of mineral oil while the solvent mixture is being distilled off at 150° C. and then at 150° C. under a vacuum of 200 torr. A sample of the interpolymer isolated from the oil has a RSV of 0.69.

#### EXAMPLE 2

50 A styrene-maleic interpolymer is obtained by preparing a solution of styrene (536 parts) and maleic anhydride (505 parts) in toluene (7585 parts) and contacting the solution at a temperature of 99°-101° C. and an absolute pressure of 480-535 mm. Hg. with a catalyst solution prepared by 55 dissolving 2.13 parts benzoyl peroxide in toluene (51.6 parts). The catalyst solution is added over a period of 1.5 hours with the temperature maintained at 99°-101° C. The mixture is maintained at 99°-101° C. and 480-535 mm. Hg. for 4 hours, then 2228 parts 40N naphthenic mineral oil 60 (Cross L-40), is added to the mixture. The resulting product is a slurry of the interpolymer in the solvent mixture. The resulting interpolymer has a reduced specific viscosity of 0.42.

#### EXAMPLE 3

65 The procedure of Example 2 is repeated employing 1.5 parts benzoyl peroxide and 2496 parts 100N mineral oil.

(including the geometric isomers thereof, i.e., cis and trans) wherein each R is independently hydrogen; halogen (e.g., chloro, bromo, or iodo); hydrocarbyl or halogen-substituted hydrocarbyl of up to about 8 carbon atoms, preferably alkyl, alkaryl or aryl; (preferably, at least one R is hydrogen, more preferably, both R are hydrogen); and each R' is independently hydrogen or lower alkyl of up to about 7 carbon atoms (e.g., methyl, ethyl, butyl or heptyl). These alpha, beta-unsaturated dicarboxylic acids, anhydrides or alkyl esters thereof contain a total carbon content of up to about 25 carbon atoms, normally up to about 15 carbon atoms. Examples include maleic anhydride; benzyl maleic anhydride; chloro maleic anhydride; heptyl maleate; itaconic anhydride; ethyl fumarate; fumaric acid, mesaconic acid; ethyl isopropyl maleate; isopropyl fumarate; hexyl methyl maleate; phenyl maleic anhydride and the like. These and other alpha, beta-unsaturated dicarboxylic compounds are 25 well known in the art. Maleic anhydride, maleic acid and fumaric acid and the lower alkyl esters thereof are preferred. Interpolymers derived from the mixtures of two or more of any of these can also be used.

Alternatively, the ester (OR') group in the above formula may contain more than 7 carbon atoms, being derived from a mixture of alcohols, some containing over 7 carbon atoms, and in such instances, the ester group may remain attached to the carboxy group during and after formation of the 30 interpolymer. This procedure provides a method of introducing the desirable ester groups initially, and eliminates the need to introduce the ester groups in a separate subsequent step.

Particularly preferred esters used in the compositions of this invention are those of interpolymers made by reacting maleic acid, or anhydride or the lower esters thereof with styrene. Of these particularly preferred interpolymers, those which are made of maleic anhydride and styrene and have a RSV in the range of about 0.08 to about 1.2, preferably about 40 0.08 to about 0.9, are especially useful. Of these latter preferred interpolymers, copolymers of maleic anhydride and styrene having a molar ratio of the maleic anhydride to styrene of about 1:1 are especially preferred. They can be prepared according to methods known in the art, as for example, free radical initiated (e.g., by benzoyl peroxide) 45 solution polymerization. Examples of such suitable interpolymerization techniques are described in U.S. Pat. Nos. 2,938,016; 2,980,653; 3,085,994; 3,342,787; 3,418,292; 3,451,979; 3,536,461; 3,558,570; 3,702,300; 3,723,375; 3,933,761; 4,284,414, and 4,604,221. These patents are incorporated herein by reference for their teaching of the preparation of suitable maleic anhydride and styrene containing interpolymers. Other preparative techniques are known in the art.

The carboxy-containing interpolymers may also be prepared using one or more additional interpolymerizable comonomer. The additional comonomer is present in relatively minor proportions. Generally, the total amount is less than about 0.3 mole, usually less than about 0.15 mole of additional comonomers for each mole of either the olefin or the alpha, beta-unsaturated carboxylic acylating agent. Examples of additional comonomers include acrylamides,

## 11

## EXAMPLE 4

The procedure of Example 1 is followed except that the interpolymer is prepared by reacting at 65°–106° C., 416 parts of styrene and 392 parts of maleic anhydride in a mixture of 2153 parts of benzene and 5025 parts of toluene in the presence of 1.2 parts of benzoyl peroxide. The resulting interpolymer has a RSV of 0.45.

## EXAMPLE 5

The procedure of Example 1 is followed except that the interpolymer is obtained by reacting at 78°–92° C., 416 parts of styrene and 392 parts of maleic anhydride in a mixture of 6106 parts of benzene and 2310 parts of toluene in the presence of 1.2 parts of benzoyl peroxide. The resulting interpolymer has RSV of 0.91.

## EXAMPLE 6

To a mixture of 392 parts of maleic anhydride in 6870 parts of benzene at 76° C. is added first 416 parts of styrene, then 1.2 parts of benzoyl peroxide. The mixture is maintained at 80°–82° C. for 5 hours. The resulting interpolymer has RSV of 1.24.

## EXAMPLE 7

The procedure of Example 6 is followed except that 1340 parts of acetone is used in place of benzene as solvent and that 0.3 parts of azobis-isobutyronitrile is used in place of benzoyl peroxide as catalyst.

## EXAMPLE 8

To a solution of 69 parts of maleic anhydride in 805 parts of benzene at 50° C. there is added 73 parts of styrene. The resulting mixture is heated to 83° C. and 0.19 parts of benzoyl peroxide is added. The mixture is then maintained at 80°–85° C., then stripped of solvent at 150° C./200 mm Hg. The resulting interpolymer has RSV of 1.64.

## EXAMPLE 9

The procedure of Example 1 is followed except that the interpolymer is prepared by the following procedure. 176 parts of maleic anhydride are dissolved in 2641 parts of xylene. To this mixture at 105° C. is added first 188 parts of styrene. Then 1.83 parts benzoyl peroxide dissolved in 32 parts xylene are added over a 1.5 hour period. The mixture is maintained at 104°–106° C. for 4 hours. The resulting interpolymer has RSV of 0.25.

## EXAMPLE 10

Heat 490 parts of maleic anhydride and 5000 parts of toluene to 100° C., then add one-half of an initiator of 2.13 parts of benzoyl peroxide in 500 parts of toluene. Add 520 parts styrene and the remainder of the initiator solution dropwise over 0.7 hour, then maintain at 100° C. for 4 hours. Theory RSV=0.30.

## EXAMPLE 11

Heat 490 parts of fumaric acid and 5000 parts of toluene to 100° C., then add one-half of an initiator solution of 4.25 parts benzoyl peroxide in 500 parts toluene. Add 520 parts of styrene and the remainder of the initiator solution dropwise over 0.7 hour, then maintain temperature at about 100° C. for 4 hours by applying a vacuum to effect reflux. Theory RSV=0.23.

## 12

## EXAMPLE 12

Mix and heat 490 parts of maleic anhydride and 5000 parts of xylene to 100° C., then add an initiator solution of 17 parts benzoyl peroxide and 500 parts xylene. Apply a vacuum to effect reflux. At 100° C. add 520 parts of styrene over 0.3 hour. The reaction is very exothermic. Maintain the reaction temperature at 100° C. for 4 hours after the addition is completed. Theory RSV=0.15.

10

## EXAMPLE 13

Mix and heat 490 parts of maleic anhydride and 6900 parts of toluene to 100° C., then add one-half of an initiator solution of 14.3 parts benzoyl peroxide and 500 parts toluene. Then add remainder of the initiator solution and a mixture of 494 parts of styrene, 29.5 parts of alpha-methyl styrene and 25 parts of methyl methacrylate dropwise over 1.5 hours. Apply a vacuum to obtain reflux at 100° C. Maintain the reaction temperature at 100° C. for 4 hours.

20 Theory RSV=0.14.

## EXAMPLE 14

Mix and heat 490 parts of maleic anhydride and 6900 parts toluene to 100° C., then add one-half of an initiator solution of 14.3 parts of benzoyl peroxide and 500 parts toluene. Apply a vacuum to obtain reflux at 100° C. Add the remainder of the initiator solution and a mixture of 494 parts of styrene and 59 parts of alpha-methyl styrene dropwise over 1.5 hours. Maintain the reaction temperature at 100° C. for 4 hours. Theory RSV=0.15.

## EXAMPLE 15

Using the same procedure as described in Example 14, polymerize 490 parts of fumaric acid with 520 parts of styrene and 29.5 parts of alpha-methyl styrene. Use 8.5 parts of benzoyl peroxide as an initiator and 7400 parts of toluene as a solvent. Theory RSV=0.20

40

## EXAMPLE 16

Repeat the procedure of Example 15 employing 17 parts of benzoyl peroxide as an initiator, Theory RSV=0.17.

45

## EXAMPLE 17

Repeat the procedure of Example 15 employing 14.3 parts of benzoyl peroxide. Theory RSV=0.14.

50

## EXAMPLE 18

Repeating the procedure of Example 15, polymerize 490 parts of maleic anhydride with 520 parts of styrene and 25 parts of methyl methacrylate using 4.3 parts of benzoyl peroxide. Theory RSV=0.26.

55

## EXAMPLE 19

Repeat the procedure of Example 18 using 8.5 part increments of benzoyl peroxide. Theory RSV=0.13.

60

## EXAMPLE 20

A reactor is charged with 1408 parts toluene and 100 parts maleic anhydride followed by heating to 95° C. With the batch refluxing at 94–96° C. a first solution of 1.68 parts benzoyl peroxide in 51 parts toluene is charged followed by the simultaneous addition over 1.5 hours of solutions of 106.1 parts styrene with 5.1 parts methyl methacrylate and 1.68 parts benzoyl peroxide in 51 parts toluene, maintaining

94–96° C. The batch is held at 94–96° C. and 440–470 mm Hg. absolute pressure for four hours until at least 97% of maleic anhydride is reacted and the RSV @ 30° C. is 0.12–0.14.

#### EXAMPLE 21

Repeat the procedure of Example 18 using 50 parts of methyl methacrylate, 8.5 parts benzoyl peroxide and 7400 parts toluene. Theory RSV=0.15.

#### EXAMPLE 22

Heat 490 parts of maleic anhydride and 5000 parts of toluene to 60° C., then add one-half of an initiator solution of 0.5 parts of Percadox 16 (Noury Chemical Company) and 500 parts of toluene. Add the styrene and the remaining initiator solution dropwise over 0.7 hour, then maintain at 60° C. for 4 hours. Theory RSV=1.5.

#### EXAMPLE 23

Mix and heat 490 parts of maleic anhydride and 6900 parts of toluene to 60° C., then add one-half of an initiator solution of 1.0 part of Percadox 16 and 500 parts of toluene. Charge the remainder of the initiator solution and a mixture of 494 parts of styrene, 29.5 parts of alpha-methyl styrene and 25 parts of methyl methacrylate dropwise over 1.5 hours, applying a vacuum to obtain reflux at 60° C. Maintain the reaction temperature at 60° C. for 4 hours. Theory RSV=0.8.

#### EXAMPLE 24

Mix and heat 490 parts of maleic anhydride and 6900 parts toluene to 60° C., then add one-half of an initiator solution of 0.5 parts Percadox 16 and 500 parts of toluene. Apply a vacuum to obtain reflux at 60° C., add the remainder of the initiator solution and a mixture of 494 parts of styrene and 59 parts of alpha-methyl styrene dropwise over 1.5 hours, then maintain at 60° C. for 4 hours. Theory RSV=1.5.

#### EXAMPLE 25

A mixture of 45.8 parts maleic anhydride and 48.64 parts styrene is charged to a reactor containing 690 parts toluene at 65° C. and mixed to form a homogeneous mixture. The temperature is adjusted to 60° C. and pressure to 140–150 mm Hg. A catalyst solution containing 0.1 part Percadox 16 in 7.2 parts toluene is added over 1.5 hours, maintaining 59°–63° C. and 140–150 mm Hg, then maintained at temperature and pressure (refluxing toluene) for 4 hours. The product is a slurry of polymer in toluene. The polymer has acid no (phenolphthalein indicator) of 3–4, indicating 95–96% conversion to polymer. The toluene mixture is transferred to a stripping vessel containing 382 parts 100N mineral oil, and stripped to 107° C. and 50 mm Hg. RSV=0.69.

#### EXAMPLE 26

The procedure of Example 25 is followed replacing the 100N mineral oil with 40N naphthenic mineral oil (Cross Oil Co.).

#### EXAMPLE 27

A reactor is charged with 794 parts C<sub>9–11</sub> substituted aromatic solvent, N<sub>2</sub> purge is begun, and the materials are heated to 65° C. whereupon 769 parts C<sub>20–24</sub> alpha-olefin and 251 parts maleic anhydride are added. The temperature

is increased to 80°, a mixture of 35.7 parts Percadox 16 in 148 parts aromatic hydrocarbon is added and the materials are heated at 80°–87° C. until the batch contains less than 0.25% maleic anhydride.

5

#### Esterification

Esterification (or transesterification, when the interpolymer contains ester groups) of the interpolymers can be accomplished by heating any of the interpolymers (having the requisite RSV) and the desired alcohol(s) and alkoxylate(s) under conditions typical for effecting esterification. Such conditions include, for example, a temperature of at least about 80° C., but more preferably from about 150° C. to about 350° C., provided that the temperature is maintained at a level below the decomposition temperature of the reaction mixture or products thereof. Water or lower alcohol is normally removed as the esterification proceeds. These conditions may optionally include the use of a substantially inert, normally liquid, organic solvent or diluent such as mineral oil, toluene, benzene, xylene or the like and an esterification catalyst such as toluene sulfonic acid, sulfuric acid, aluminum chloride, boron trifluoride-triethylamine, methane sulfonic acid, hydrochloric acid, ammonium sulfate, phosphoric acid, sodium methoxide or the like.

20

25 These conditions and variations thereof are well known in the art.

When the ester is a non-nitrogen-containing ester, it is preferable that substantially all the carboxy functions of the interpolymers be reacted with the alcohols and alkoxylates. Nevertheless, useful products can be obtained when at least about 50%, preferably at least about 70%, more preferably at least about 90% and advantageously at least about 95% of the carboxy functions have been so reacted. An excess of alcohols and alkoxylates over the stoichiometric requirement for complete esterification of the carboxy functions is often used. As a practical matter, however, complete esterification may be too difficult or time consuming to achieve. While excess (over stoichiometric requirement) of alcohols and alkoxylates or unreacted alcohols and alkoxylates need not be removed as such alcohols and alkoxylates can serve, for example, as diluent or solvent in the use of the esters, and similarly, optional reaction media, e.g., toluene, need not be removed as they can similarly serve as diluent or solvent in the use of the esters, it is generally preferred that unreacted alcohols, alkoxylates and diluents are removed by techniques, such as distillation, etc., that are well-known in the art.

40

45 As noted above, the compositions of this invention contain ester groups. Esters (I) and (III) each contain ester groups consisting essentially of those having at least 8 carbon atoms. The ester groups are formed by reacting the carboxy-containing interpolymer with an alcohol. The alcohol generally contains at least 7 carbon atoms. In one embodiment, the alcohol contains from about 7, or about 8 to about 30, or to about 24, or even to about 18 carbon atoms. Examples of useful alcohols include heptanol, octanol, decanol, dodecanol, tridecanol, pentadecanol, octadecanol, etc.

50

55 One class of alcohols includes commercially available mixtures of alcohols. These include oxoalcohols which comprise, for example, a mixture of alcohols having from about 8–24 carbon atoms. Of the various commercial alcohols, another class of alcohols includes the alcohols having from about 8 to 30 aliphatic carbon atoms. The alcohols may comprise, for example, octyl alcohol, decyl alcohol, dodecyl alcohol, tetradecyl alcohol, pentadecyl

60

65 One class of alcohols includes commercially available mixtures of alcohols. These include oxoalcohols which comprise, for example, a mixture of alcohols having from about 8–24 carbon atoms. Of the various commercial alcohols, another class of alcohols includes the alcohols having from about 8 to 30 aliphatic carbon atoms. The alcohols may comprise, for example, octyl alcohol, decyl alcohol, dodecyl alcohol, tetradecyl alcohol, pentadecyl

alcohol, eicosyl alcohol, octadecyl alcohol, etc. Several suitable sources of these alcohol mixtures are the technical grade alcohols sold under the name Neodol® alcohols (Shell Oil Company, Houston, Tex.) and under the name Alfol® alcohols (Vista Chemical, Westlake, La.), and fatty alcohols derived from animal and vegetable fats and sold commercially by, for example, Henkel, Condea, and Emory.

Esters (II) and (IV) are mixed esters derived from a combination of alcohols including alcohols containing at least 7 carbon atoms (relatively high molecular weight alcohols) and alcohols containing less than 7 carbon atoms (relatively low molecular weight alcohols). Alcohols containing at least 7 carbon atoms are those described hereinabove. Alcohols containing less than 7 carbon atoms generally contain from 1, or about 2, to about 6, or to about 5 carbon atoms. Examples of the low molecular weight alcohols include methanol, ethanol, propanol, butanol, pentanol, hexanol, cyclopentanol, and cyclohexanol. The above list is also meant to include the various isomeric arrangements of these alcohols. For instance, butanol refers to n-butanol, sec-butanol, isobutanol, etc.

Mixed esters of the carboxy-containing interpolymer are most conveniently prepared by first esterifying the carboxy-containing interpolymer with a relatively high molecular weight alcohol and a relatively low molecular weight alcohol to convert at least about 50%, or about 70% up to about 95%, or to about 98% up to about 100% of the carboxy groups of the interpolymer to ester groups. Nitrogen-containing esters are prepared by neutralizing any remaining carboxy groups with ammonia, an amine, or a hydrazine such as those described below to obtain nitrogen-containing esters.

To incorporate the appropriate amounts of the two alcohol groups into the polymer to form mixed esters, the ratio of the high molecular weight alcohol to the low molecular weight alcohol used in the process should be within the range of from about 2:1 to about 9:1 on a molar basis. In most instances, the ratio is from about 2.5:1 to about 5:1.

When utilizing a combination of a high molecular weight alcohol and a low molecular weight alcohol, the esterification may be carried out, for example, by initially esterifying at least about 50 molar percent or from about 50 to 75 molar percent, frequently up to about 90 molar percent of the carboxy radicals with the high molecular weight alcohol and then subsequently esterifying the partially-esterified carboxy-containing interpolymer with a low molecular weight alcohol, e.g., 2-4 carbon atoms, to obtain a carboxy interpolymer having approximately 50-90 molar percent of the carboxylic groups esterified with the high molecular weight aliphatic alcohol and approximately 8-48 molar percent of the carboxy radicals esterified with the low molecular weight aliphatic alcohol. For example, esterification with a combination of high and low molecular weight alcohols may be accomplished, in sequence, by first carrying out the esterification with the high molecular weight alcohol, e.g., up to about 75 molar percent and subsequently esterifying the remaining carboxylic groups with the low molecular weight alcohol, to attain the desired degree of esterification.

Alternatively, the carboxylic groups of the interpolymer may be simultaneously esterified with a mixture of the alcohols to obtain an esterified carboxy-containing interpolymer having up to about 60, or to about 70, or to about 80, or to about 90, or to about 95 or to about 98 mole percent, up to 100%, of the carboxylic groups esterified with combination of high and low molecular weight aliphatic alcohols.

In another embodiment, the carboxy-containing interpolymers contains a carbonyl-amino group. The carbonyl-amino groups include amides, imides, amidines, ammonium salts, amidic acid salts or mixtures thereof. A carbonyl-amino group is derived from the carboxy group of the carboxy-containing interpolymer and an amine. The carbonyl-amino group may be present when the carboxy-containing interpolymer contains esters derived from a single alcohol or mixtures of alcohol as described above.

10 Unesterified carboxylic groups of the interpolymer may be converted to carbonyl-amino groups by reaction with ammonia or an amine. The amines which are used to form carbonyl-amino group may be mono- or polyamines provided that the average number of primary and secondary amino nitrogens range from about 1 to about 1.1. To illustrate, the amine may be a monoamine containing one primary or secondary amino group. Here the number of primary or secondary amino groups is 1. The amine may be a polyamine, wherein one amino group is primary or secondary and one or more is tertiary. Aminopropylmorpholine is an example. The amine reactant may also be a mixture of these with one or more polyamines containing 2 or more primary or secondary amino groups, provided that the average number of primary or secondary amino groups is no greater than about 1.1.

25 Examples of monoamines include aliphatic amines such as mono-, di- and tri-alkyl amines having alkyl groups containing from 1 to about 20 carbon atoms as well as cyclic monoamines. In one embodiment, the amines are 30 polyamines having from 1 to about 1.1, preferably one, primary or secondary amino group, and at least one mono-functional amino group such as a tertiary-amino group or heterocyclic amino group derived from pyrroles, pyrrolidones, caprolactams, oxazolidones, oxazoles, 35 thiazoles, pyrazoles, pyrazolines, imidazoles, imidazolines, thiazines, oxazines, diazines, oxacarbamyl, thiocarbamyl, uracils, hydantoin, thiohydantoin, guanidines, ureas, sulfonamides, phosphoramides, phenothiazines, amidines, etc. In one embodiment, the carbonyl-polyamino group is 40 derived from a morpholine. Examples of morpholines include aminoethylmorpholine, aminopropylmorpholine, etc. Examples of such polyamines include dimethylaminoethylamine, dibutylamino-ethylamine, 3-dimethylamino-1-propylamine, 4-methylethylamino-1-butylamine, pyridylethylamine, N-morpholinoethylamine, tetrahydropyridylethylamine, bis-(dimethylamino)propylamine, bis(diethylamino)ethylamine, N,N-dimethyl-p-phenylene diamine, piperidyl-ethylamine, 1-aminoethylpyrazone, 1-(methyl-amino)pyrazoline, 1-methyl-4-aminoctyl 45 pyrazole, 1-mninobutylimidazole, 4-aminoethylthiazole, 2-aminoethyltriazine, dimethylcarbamylpropylamine, N-methyl-N-aminopropylacetamide, N-aminoethylsuccinimide, N-methylamino-maleimide, N-aminoethylalpah-chlorosuccinimide, 3-aminoethyluracil, 50 2-amino-ethylpyridine, ortho-aminoethyl-N,N-dimethylbenzenesulfamide, N-aminoethyl-phenothiazine, N-aminoethylacetamide, 1-aminophenyl-2-methylimidazoline, N-methyl-N-aminoethyl-S-ethylthiocarbamate, etc. For the most part, the amines are 55 those which contain only one primary-amino or secondary-amino group and, preferably at least one tertiary-amino group. The tertiary amino group is preferably a heterocyclic amino group. In some instances polyamines may contain up to about 6 amino groups although, in most instances, they 60 contain one primary-amino group and either one or two tertiary-amino groups. The polyamines may be aromatic or aliphatic mines and are preferably heterocyclic amines such 65

as aminoalkyl-substituted morpholines, piperazines, pyridines, benzopyrroles, quinolines, pyrroles, etc. They are usually amines having from 4 to about 30, or to about 12 carbon atoms. Polar substituents may likewise be present in the amines.

The carbonyl-amino groups of the carboxy-containing interpolymers also may comprise the groups derived from hydrazine and/or a hydrocarbon-substituted hydrazine including, for example, the mono-, di-, tri-, and tetrahydrocarbon-substituted hydrazines wherein the hydrocarbon substituent is either an aliphatic or aromatic substituent including, for example, the alkyl, e.g., cyclic and/or acyclic groups, aryl-, alkylaryl-, aralkyl, etc. The hydrocarbon substituents, generally, contain from 1, up to about 24 or up to about 12 aliphatic carbon atoms. The preferred substituents, however, include for example, phenyl, alkylphenyl or an alkyl group wherein the alkyl group is either a methyl, ethyl, propyl, butyl, pentyl, octyl, cyclohexyl, decyl or dodecyl group. Other examples of the hydrocarbon groups include octyldecyl, behenyl, benzyl, heptaphenyl, alpha-naphthyl, beta-naphthyl, butyl-naphthyl, oleyl, and stearyl groups. Of the various hydrocarbon-substituted hydrazines, a preferred class includes the N,N-dihydrocarbon-substituted hydrazines, e.g., the dimethyl, diethyl, diphenyl and dibutyl hydrazines.

In the embodiment where the carboxy-containing interpolymer is characterized as containing a carbonyl-amino group, the carboxy-containing interpolymer may be esterified as described above. Following esterification of the carboxy groups of the interpolymer with either one or more of the high and low molecular weight alcohols, at least about 2 molar percent, or from about 2, or about 5, up to 50, or to about 5 molar percent of the carboxy groups of the interpolymer may be reacted with an amine at temperatures ranging from about 80°-300° C., up to 350° C. or higher provided that said temperature is maintained below the decomposition point of either the reactants and the products obtained thereof. Thus, for example, at least about 50 mole percent, e.g., 50-98 mole percent, of the carboxy groups of a carboxy-containing interpolymer may be esterified with a high molecular weight aliphatic alcohol and then subsequently reacted with a amine, to obtain a nitrogen-containing ester having about 2 to about 50 or to about 35 molar percent of the carboxylic groups converted to carbonyl-amino groups. If a mixture of alcohols including the high molecular weight and low molecular weight alcohols is used to esterify the carboxyl groups of said interpolymer, then at least about 2 molar percent of the carboxyl groups of said interpolymer are reacted with the amine, to obtain the carbonyl-amino groups. The amount of amine is sufficient to neutralize substantially all of the unesterified carboxy groups of the polymer. An excess of amine may be used.

In another embodiment, the carboxy-containing interpolymer is reacted with a relatively high molecular weight alcohol, a relatively low molecular weight alcohol and an amine. The alcohols and amines have been described above. The alcohols may be reacted with the interpolymer to form an intermediate which is subsequently reacted with the amine. Alternatively the alcohols and amine may be reacted with the interpolymer simultaneously. For convenience, the relative proportions of the high molecular weight ester group to the low molecular weight ester group and to the carbonyl-amino group are expressed in terms of molar ratios of (60-94):(5-30):(1-15), respectively. The preferred ratio is (70-90):(10-25):5.

#### Examples of Esterification of the Interpolymer

The following examples serve to illustrate the preparation of the esters and nitrogen-containing esters of the carboxy-

containing interpolymers used in this invention and are not intended as limiting thereof. Unless otherwise indicated in these and the following examples, or in the specification, all parts and percentages are by weight, and temperatures are in degrees Celsius. Sulfuric acid is typically commercially available 93-96% H<sub>2</sub>SO<sub>4</sub>. Methanesulfonic acid is nominally 70% in H<sub>2</sub>O. The extent of esterification is calculated by determining the total acid number (phenolphthalein indicator) and the strong acid number (bromphenol blue indicator) of the reaction mixture. The total acid number includes contributions from unesterified polymer and catalyst. The strong acid number is the measure of the acid number of the catalyst. The difference between the two acid numbers, the net acid number, is the acid number due to unesterified polymer.

#### EXAMPLE 1-E

To 209 parts of the stripped mineral oil-interpolymer slurry of Example 1 there are added 25.2 parts toluene, 4.8 parts n-butyl alcohol, 56.6 parts of a commercial alcohol consisting essentially of primary alcohols having from 12 to 18 carbon atoms and 10 parts of a commercial alcohol consisting of primary alcohols having from 8 to 10 carbon atoms and to the resulting mixture there is added 2.3 parts sulfuric acid. The mixture is then heated at 150°-160° C. for 20 hours whereupon water is distilled off. An additional 0.18 part of sulfuric acid together with an additional 3 parts of n-butyl alcohol is added and the esterification is continued until 95% of the carboxy radicals of the polymer has been esterified.

#### EXAMPLE 2-E

The procedure of Example 1-E is followed except that the esterification is carried out in two steps, the first step being the esterification of the styrene-maleic interpolymer with the commercial alcohols having from 8 to 18 carbon atoms and the second step being the further esterification of the interpolymer with n-butyl alcohol.

#### EXAMPLE 3-E

The procedure of Example 1-E is followed except that the esterification is carried out by first esterifying the styrene-maleic interpolymer with the commercial alcohols having from 8 to 18 carbon atoms until 70% of the carboxyl radicals of the interpolymer have been converted to ester radicals and thereupon continuing the esterification with any yet-unreacted commercial alcohols and n-butyl alcohol until 95% of the carboxyl radicals of the interpolymer have been converted to ester radicals.

#### EXAMPLE 4-E

The procedure of Example 1-E is followed employing the interpolymer of Example 3.

#### EXAMPLE 5-E

The procedure of Example 1-E is followed employing the interpolymer of Example 4.

#### EXAMPLE 6-E

The procedure of Example 1-E is followed employing the interpolymer of Example 5.

#### EXAMPLE 7-E

The procedure of Example 6-E is followed employing the interpolymer of Example 6.

19

## EXAMPLE 8-E

The procedure of Example 1-E is followed employing the interpolymer of Example 7.

## EXAMPLE 9-E

The procedure of Example 1E is followed except that 3.5 parts of toluene sulfonic acid is used in place of sulfuric acid as the esterification catalyst.

## EXAMPLE 10-E

The procedure of Example 1E is followed except that 2.5 parts of phosphoric acid is used in place of sulfuric acid as the esterification catalyst.

## EXAMPLE 11-E

The procedure of Example 1E is followed except that dodecyl alcohol (0.7 mole per carboxy equivalent of the styrene-maleic anhydride interpolymer) is used in place of the alcohol mixtures having 8 to 18 carbon atoms and isobutyl alcohol (0.2 mole per carboxy equivalent of the interpolymer) is used in place of n-butyl alcohol.

## EXAMPLE 12-E

The procedure of Example 1E is followed except that eicosyl alcohol (0.8 mole consumed per carboxy equivalent of interpolymer) is used in place of the commercial alcohols having from 8 to 18 carbon atoms and n-pentyl alcohol (0.15 mole consumed per carboxy equivalent of the interpolymer) is used in place of the n-butyl alcohol.

## EXAMPLE 13-E

A mixture of 4554 parts of the interpolymer oil solution of Example 2, 1525 parts of a behenyl alcohol mixture provided by Henkel (a mixture of 17.4 mole percent of  $C_{18}$  primary alcohol, 15.6 mole percent of  $C_{20}$  primary alcohol, and 67 mole percent of  $C_{22}$  primary alcohol), 416 parts of Aifonic 1412-40, a product of Conoco identified as an ethoxylate of the formula



73 parts of para-toluene sulfonic acid and 18.6 parts of an isomeric mixture of butylphenol is heated to a temperature of 105° C. over a period of 1.75 hours with stirring and nitrogen blowing at one standard cubic foot per hour. The reaction mixture begins to reflux steadily. The temperature is raised to 150° C. over a period of 3.5 hours. 3463 parts of azeotrope are collected. The nitrogen blowing rate is reduced to 0.3 cubic foot per hour. The reaction mixture is maintained at 150° C. for 18 hours. 350 parts of xylene are added to the reaction mixture with stirring, and the reaction mixture is maintained at 150° C. for two hours. 303 parts of xylene are added to the reaction mixture, and distillation of remaining toluene in the reaction mixture is commenced. After 2.25 hours of continued heating at 150° C., 355 parts xylene are added. After 0.75 hour of continued heating at about 148° C., 423 parts of xylene are added. After 0.25 hour of heating at 148° C., 360 parts of xylene are added. After an additional 0.5 hour of maintaining the reaction mixture at 148° C., heating is discontinued. At this point, the total amount of azeotrope collected is 4304 pans. The reaction mixture is cooled to 95° C. 3847 parts of the reaction mixture are diluted with 1219 parts of xylene to provide the desired product.

## EXAMPLE 14-E

A mixture of 613 parts of the interpolymer oil slurry of Example 2, 201 parts of the behenyl alcohol mixture iden-

20

tified in Example 13-E, 16 parts of an isomeric mixture of  $C_{13}$  alkanols, 27.2 parts of Aifonic 1412-40, 11 parts of paratoluene sulfonic acid, and 2 parts of an isomeric mixture of butyl phenol is stirred and heated to reflux under nitrogen blowing at one standard cubic foot per hour. 358 parts of azeotrope are removed, the remaining mass being 512 pans. The reaction mixture temperature is increased to 152° C. The rate of nitrogen blowing is reduced to about 0.1 cubic foot per hour. The reaction mixture is maintained under reflux conditions for about 26 hours. The reaction mixture is then cooled to 100° C. and 143 parts of xylene are added to the reaction mixture to provide the desired product.

## EXAMPLE 15-E

15 A toluene slurry (2057 parts), having 11.06% solids and 88.94% volatiles, of the maleic anhydride/styrene interpolymer of Example 2, 631 parts Neodol 45, a product of Shell Chemical Company identified as a mixture of  $C_{14}$  and  $C_{14}$  linear primary alcohols, 750 parts mineral oil, and 4.2 parts 20 Ethyl Antioxidant 733, a product of Ethyl identified as an isomeric mixture of butyl phenols, are charged to a vessel. The mixture is heated with medium agitation under nitrogen purge at 0.5 standard cubic feet per hour until the temperature reaches 155° C. 10.53 parts methane sulfonic acid catalyst in water is added dropwise over period of 20 minutes. Nitrogen purge is increased to 1.0 cubic foot per hour and temperature is raised by removal of toluene-water distillate. The mixture is maintained at a temperature of 150° C. for five hours under a nitrogen purge of 0.1-0.2 standard cubic feet per hour. 15.80 parts additional methanesulfonic acid solution is added to the mixture over 0.25 hours. The mixture is maintained at 150° C. for 3.5 hours. The degree of esterification is 95.08%. The materials are vacuum stripped.

## EXAMPLE 16-E

A reactor is charged with 416 parts of the toluene-oil slurry of Example 3 and 228 parts Neodol 45L followed by 40 heating to 115° C. whereupon 35 parts methanesulfonic acid are added over 0.3 hour. The temperature is increased to 150° C. while removing water and excess toluene, the materials are held at 150° C. for 5 hours then an additional 1 parts methanesulfonic acid is added over 0.25 hour 45 followed by additional heating for 3.5 hours until net acid number indicates 95% esterification. The materials are stripped and filtered.

## EXAMPLE 17-E

50 The procedure of Example 15-E is repeated with the exception that both Neodol 45 (315.4 parts) and Alfol 1218 (312.5 parts), a product of Vista Chemical identified as a mixture of synthetic primary straight chain alcohols having 12 to 18 carbon atoms, are initially charged, rather than 631 parts of Neodol 45 which were included in the initial charge in Example 15-E.

## EXAMPLE 18-E

60 A toluene slurry (1125 parts), having 13.46% solids and 86.54% volatiles, of the maleic anhydride/styrene interpolymer of Example 2, 350 parts mineral oil and 344 parts Neodol 45 are charged to a vessel. The mixture is heated with medium agitation under nitrogen sweep of 0.5 cubic feet per hour until the temperature reaches 110° C. 8.55 parts paratoluene sulfonic acid in 9 parts water is added dropwise over a period of 0.4 hour. The temperature of the mixture is

increased to 152° C. by removing toluene-water distillate. The temperature is maintained at 152°–156° C. under nitrogen sweep of 0.5 standard cubic feet per hour until the net acid number indicates that esterification is at least 95% complete. The materials are vacuum stripped.

#### EXAMPLE 19-E

The procedure of Example 17-E is repeated with the exception that both Neodol 45 (172 parts) and Alfol 1218 (169 parts) are provided in the initial charge, rather than the 344 parts of Neodol 45 provided in Example 17-E.

#### EXAMPLE 20-E

The product of Example 2 (101 parts), Neodol 91 (56 parts), a product of Shell Chemical Company identified as a mixture of C<sub>9</sub>, C<sub>10</sub> and C<sub>11</sub> alcohols, TA-1618 (92 parts), a product of Proctor & Gamble identified as a mixture of C<sub>16</sub> and C<sub>18</sub> alcohols, Neodol 25 (62 parts), a product of Shell Chemical Company identified as a mixture of C<sub>12</sub>, C<sub>13</sub>, C<sub>14</sub>, and C<sub>15</sub> alcohols, and toluene and the contents are heated. Methane sulfonic acid (5 parts) is added to the mixture. The mixture is heated under reflux conditions for 30 hours. The materials are vacuum stripped conditions for 30 hours. The materials are vacuum stripped.

#### EXAMPLE 21-E

The product of Example 2 (202 parts), Neodol 91 (112 parts), TA 1618 (184 parts), Neodol 25 (124 parts) and toluene (875 parts) are charged to a vessel. The mixture is then heated and stirred. Methanesulfonic acid (10 parts) is added to the mixture which is then heated under reflux conditions for 31 hours. The materials are vacuum stripped.

#### EXAMPLE 22-E

The product of Example 2 (101 parts), Alfol 810 (50 parts), a product of Vista Chemical identified as a mixture of C<sub>8</sub> and C<sub>10</sub> alcohols, TA-1618 (92 parts), Neodol 25 (62 parts) and toluene (437 parts) are charged to a vessel. The mixture is heated and stirred. Methanesulfonic acid (5 parts) is added to the mixture which is heated under reflux conditions for 30 hours. The materials are vacuum stripped.

#### EXAMPLE 23-E

A reactor is charged with 389 parts of the toluene-oil slurry of Example 2 and 103 parts of Alfol 1218, the mateddais are heated to 95° C. under N<sub>2</sub> whereupon a solution of 5.5 parts methanesulfonic acid in 68 parts Alfol 8-10 is charged. The material are heated to 150° C. while removing water of esterification and excess toluene, the reaction is continued for 5 hours followed by addition over 0.25 hour of 3.7 parts butanol. The materials are refluxed until the net acid number indicates at least 95% esterification. The materials are stripped and filtered.

#### EXAMPLE 24-E

A toluene slurry (799 parts) of a maleic anhydride/styrene interpolymer (11.82% polymer, RSV=0.69) is charged to a vessel. The vessel is purged with nitrogen while stirring the contents for 15 minutes. Alfol 1218 (153 parts), Neodol 45 (156 parts) and sulfuric acid (5 parts) are added to the mixture, then 125 parts toluene. The mixture is heated at 150°–156° C. for 18 hours. The materials are vacuum stripped.

#### EXAMPLE 25-E

A toluene slurry (973 parts) of a maleic anhydride/styrene interpolymer (17.28% solids, RSV=0.69) is charged to a

vessel. The slurry is stirred and blown with nitrogen at 0.75–1.0 cubic feet per hour for 20 minutes. Neodol 45 (368 parts) and 6.84 parts 80% sulfuric acid are added to the mixture. The mixture is heated at 150°–156° C. for 23 hours.

5 Additional 80% sulfuric acid (1 part) and 50 parts toluene are added after approximately the first 9 hours of heating. Additional 80% sulfuric acid (2.84 parts) is added after about the first 13 hours of heating. Additional Neodol 45 (18.4 parts) and 80% sulfuric acid (2 parts) are added after 10 about the first 16 hours of heating. The materials are vacuum stripped.

#### EXAMPLE 26-E

A toluene and mineral oil slurry (699 parts) containing 15 17.28% solids of a maleic anhydride/styrene interpolymer (reduced specific viscosity of 0.69), Neodol 45 (139 parts), Alfol 1218 (138 parts), Ethyl Antioxidant 733 (2.9 parts) and toluene (50 parts) are charged to a vessel. The mixture is heated under a nitrogen purge at 0.5 standard cubic feet per hour. Methane sulfonic acid (3.9 parts) is added dropwise over a period of 9 minutes. The mixture is heated under reflux conditions for 35 minutes. Toluene (51 parts) is added to the mixture which is then heated for an additional 3 hours 20 15 minutes under reflux conditions. Methane sulfonic acid (3 parts) is added dropwise over a period of 3 minutes. The mixture is heated under reflux conditions for 3 hours 15 minutes. Methane sulfonic acid (3.9 parts) is added dropwise over a period of 12 minutes. The mixture is heated at 150°–152° C. for 3 hours 45 minutes. The materials are 25 vacuum stripped.

#### EXAMPLE 27-E

Charge a vessel with a slurry (870 parts) having 15.5% 35 solids and 84.5% volatiles of the interpolymer of Example 9 and 278 parts Alfol 1218. Heat the mixture to 100° C. under nitrogen with medium agitation. Add 3.1 parts sulfuric acid and 48.7 parts of Alfol 810. Raise the temperature of the mixture to 145° C.–150° C. by removing toluene-water 40 distillate. Add 301 parts of a mineral oil. Maintain the temperature of the mixture at 145° C.–150° C. for 6 hours. Add 54 parts mineral oil. Maintain at 145° C.–150° C. until net acid number indicates that esterification is at least 75% 45 complete. Add 26.7 parts of n-butanol dropwise over 15 minutes. Maintain the temperature of the mixture at 145° C.–150° C. for 3 hours. Add solution of 0.52 parts sulfuric acid and 26.7 parts of butanol dropwise over 10 minutes. Maintain the temperature of the mixture at 145° C.–150° C. until the net acid number indicates that the esterification is 50 at least 95% complete. Add sodium hydroxide (0.96 parts of a 50% aqueous solution) to the mixture, then 1.36 parts Ethyl Antioxidant 733. Vacuum strip the mixture at 155° C. and 5 mm Hg. Add 10 parts diatomaceous earth to the mixture along with 1.36 parts Ethyl Antioxidant 733. Cool to 100° C. and filter through a heated funnel.

#### EXAMPLE 28-E

Esterify a toluene slurry (928 parts) having 15.5% solids 60 and 84.5% volatiles of the interpolymer of Example 10 utilizing the same procedure as Example 27-E. Use 348 parts Alfol 1218, 16 parts Alfol 810, 4.53 parts of sulfuric acid, 293 parts of a mineral oil, 66.6 parts of butanol, 1.46 parts of Ethyl Antioxidant 733 and 10 parts of diatomaceous earth.

#### EXAMPLE 29-E

Charge to a suitable vessel 404 parts of the interpolymer 65 slurry of Example 12 and 555 parts Alfol 1218. Heat the

mixture to 100° C. with agitation under nitrogen. Add Alfol 810 (98 parts) and methanesulfonic acid (6.4 parts) to the mixture. Raise the temperature to 150° C. by removal of water-xylene distillate. Maintain the temperature of the mixture at 150° C. until net acid number indicates that esterification is at least 75% complete. Add butanol (104 parts) dropwise to the mixture. Maintain the temperature of the mixture at 150° C. until the net acid number indicates that esterification is at least 95% complete. Add Ethyl Antioxidant 733 (4.6 parts) and 2 parts 50% aqueous sodium hydroxide to the mixture, mix, then vacuum strip at 150° C. and 20 mm Hg. Cool to 100° C., add 4.6 parts Ethyl Antioxidant 733 and 36 parts diatomaceous earth then filter through a heated funnel.

## EXAMPLE 30-E

Charge to a suitable vessel a toluene slurry (1688 parts) having 12.32% solids and 87.68% volatiles of the interpolymer of Example 13, 257 parts Alfol 1218 and 130 parts mineral oil. Heat the mixture to 100° C. with medium agitation under nitrogen. Add 4.22 parts sulfuric acid and 45 parts Alfol 810 to the mixture. Heat the mixture to 150° C. by removing toluene-water distillate. Add 27 parts butanol to the mixture. Maintain the temperature of the mixture at 150° C. for 1½ hours. Add a second portion of 27 parts butanol to the mixture. Maintain the temperature of the mixture at 150° C. until the net acid number indicates that esterification is at least 95% complete. Add sodium hydroxide (1.44 parts of a 50% aqueous solution) and 1.04 parts Isonox 133 (Schenectady Chemicals, Freeport, Tex.) to the mixture. Vacuum strip the mixture at 150° C. and 100 torr. Add a second portion of Isonox 133 (1.04 parts) along with diatomaceous earth (16 parts). Cool the mixture to 100° C. and filter through a hot funnel.

## EXAMPLE 31-E

Esterify 208 parts of the interpolymer of Example 14 by the same procedure as Example 28-E. Use 257 parts of Alfol 1218, 45 parts of Alfol 810, 130 parts of mineral oil, 4.22 parts of sulfuric acid, 54 parts of butanol, 1.28 parts of a 50% aqueous solution of sodium hydroxide, 2 parts of Isonox 133 and 16 parts of diatomaceous earth.

## EXAMPLE 32-E

Esterify 208 parts of the interpolymer of Example 15 by the same procedure as Example 28-E. Use 257 parts of Alfol 1218, 45.2 parts of Alfol 810, 222 parts of mineral oil, 4.22 parts of sulfuric acid, 54 parts of butanol, 2 parts of a 50% aqueous sodium hydroxide solution, 2.22 parts of Isonox 133 and 15 parts of diatomaceous earth.

## EXAMPLE 33-E

Esterify the interpolymer of Example 16 by the same procedure as 28-E. Use 278 parts of Alfol 1218, 49 parts of Alfol 810, 136 parts of a mineral oil, 4.21 parts of sulfuric acid, 54 parts butanol, 1.14 parts of a 50% aqueous sodium hydroxide solution, 2.08 parts of Isonox 133 and 16 parts of diatomaceous earth.

## EXAMPLE 34-E

Esterify the interpolymer of Example 17 by the same procedure as 28-E. Use 257 parts of Alfol 1218, 45 parts of Alfol 810, 310 parts of a mineral oil, 4.2 parts of sulfuric acid, 54 parts butanol, 1.21 parts of a 50% aqueous sodium hydroxide solution, 2 parts of Isonox 133 and 16 parts of diatomaceous earth.

## EXAMPLE 35-E

Esterify the interpolymer of Example 18 by the procedure utilized in Example 28-E. Use 278 parts of Alfol 1218, 49 parts of Alfol 810, 362 parts of a mineral oil, 4.21 parts of sulfuric acid, 54 parts butanol, 1.28 parts of a 50% aqueous sodium hydroxide solution, 1.72 parts of Isonox 133 and 20 parts of diatomaceous earth.

## EXAMPLE 36-E

10 Esterify the interpolymer of Example 19 utilizing the procedure described in Example 28-E. Use 257 parts of Alfol 1218, 45.2 parts of Alfol 810, 134 parts of a mineral oil, 54 parts butanol, 2.05 parts of a 50% aqueous sodium hydroxide solution, 2.08 parts of Isonox 133 and 16 parts of diatomaceous earth. Replace the sulfuric acid of Example 28-E with 5.46 parts of methanesulfonic acid.

## EXAMPLE 37-E

20 A reactor is charged with 815 parts of the terpolymer slurry of Example 20 and 65 parts Cross Oil Co. L-40. The mixture is stripped to remove toluene followed by addition of 104.4 parts Alfol 1218, the batch is heated to 96° C. then 5.3 parts of methanesulfonic acid and 49 parts Alfol 8-10 are charged followed by heating to 146° C. The batch is held at 146°-152° C. until the acid no is between 19-21 whereupon 10.7 parts butanol are added. The reaction is continued until the acid number is 5-6, then 1.1 parts 50% aqueous NaOH are added followed by mixing for 1 hour at 150° C. The material are vacuum stripped then filtered.

## EXAMPLE 38-E

25 Esterify 212 parts of the interpolymer of Example 21 according to the procedure as described in Example 28-E, except use 5.46 parts of methanesulfonic acid in place of sulfuric acid. Use 278 parts of a mineral oil, 54 parts of butanol, 2 parts of a 50% aqueous sodium hydroxide solution, 2.08 parts of Isonox 133 and 16 parts of diatomaceous earth.

## EXAMPLE 39-E

30 Esterify the interpolymer of Example 22 by the same procedure as 30-E. Use 257 parts of Alfol 1218, 45 parts of Alfol 810, 130 parts of a mineral oil, 4.2 parts of sulfuric acid, 54 parts butanol, 1.21 parts of a 50% aqueous sodium hydroxide solution, 2 parts of Isonox 133 and 16 parts of diatomaceous earth.

## EXAMPLE 40-E

35 Esterify the interpolymer of Example 23 utilizing the procedure described in Example 30-E. Use 257 parts of Alfol 1218, 45.2 parts of Alfol 810, 134 parts of a mineral oil, 54 parts butanol, 2.05 parts of a 50% aqueous sodium hydroxide solution, 2.08 parts of Isonox 133 and 16 parts of diatomaceous earth. Replace the sulfuric acid of Example 30-E with 5.46 parts of methanesulfonic acid.

## EXAMPLE 41-E

40 Esterify 212 parts of the interpolymer of Example 24 according to the procedure as described in Example 28-E, except use 5.46 parts of a solution of methanesulfonic acid in place of sulfuric acid. Use 278 parts of Alibi 1218, 49 parts of Alfol 810, 136 parts of a mineral oil, 54 parts of butanol, 2 parts of a 50% aqueous sodium hydroxide solution, 2.08 parts of Isonox 133 and 16 parts of diatomaceous earth.

## EXAMPLE 42-E

Charge to a suitable vessel a toluene slurry (1688 parts) having 12.32% solids and 87.68% volatiles of the interpolymer of Example 10, Alfol 1218 (217 parts) and mineral oil (130 parts). Heat the mixture to 100° C. with medium agitation under nitrogen. Add 4.22 parts sulfuric acid and 101 parts Alfol 810 to the mixture. Heat the mixture to 150° C. by removing toluene-water distillate. Add 20 parts butanol to the mixture. Maintain the temperature of the mixture at 150° C. for 1½ hours. Add a second portion of 20 parts butanol to the mixture. Maintain the temperature of the mixture at 150° C. until the net acid number indicates that esterification is at least 95% complete. Vacuum strip the mixture at 150° C. and 100 mm Hg. Cool the mixture to 100° C. and filter through a hot funnel.

## EXAMPLE 43-E

Charge to a suitable vessel 404 parts of the interpolymer of Example 12 and 555 parts Alfol 1218. Heat the mixture to 100° C. with agitation under nitrogen. Add 98 parts Alfol 810 and 6.4 parts methanesulfonic acid to the mixture. Raise the temperature to 150° C. by removal of water-xylene distillate. Maintain the temperature of the mixture at 150° C. until net acid number indicates that esterification is at least 75% complete. Add 104 parts butanol dropwise. Maintain the temperature at 150° C. until net acid number indicates that esterification is at least 95% complete. Vacuum strip the mixture at 150° C. and 20 mm Hg. Cool the mixture to 100° C. and add 36 parts diatomaceous earth. Filter the mixture through a heated funnel.

## EXAMPLE 44-E

A reactor is charged with a slurry of the copolymer of Example 25 which contains 100 parts polymer, 412 parts 100N oil and 44 parts toluene. To the slurry are added 124.2 parts EPAL 1214 (Albermarle Chemical, Baton Rouge, La.) 13.8 parts Alfol 1218 and 8.3 parts 100N mineral oil, then 12.2 parts Alfol 8-10. The materials are mixed then a mixture of 2 parts 93% sulfuric acid in 12.2 parts Alfol 8-10 is added followed by heating to boiling at 150° C. and the reaction is continued at 150°-160° C. while azeotroping water of reaction for 2.5 hours until the polymer has been 75% esterified. A first mixture of 13.3 parts butanol and 0.55 parts H<sub>2</sub>SO<sub>4</sub> is added and the reaction is continued at temperature for 2.5 hours until acid number is 11-13 indicating about 85% conversion. whereupon a second identical mixture of butanol and H<sub>2</sub>SO<sub>4</sub> is added. Reaction is continued at temperature for 5.5 hour until 95% conversion is attained. The material is stripped and filtered.

## EXAMPLE 45-E

A reactor is charged with the slurry of Example 26 which contains 100 parts of polymer, 412.5 parts Cross L-40 oil and 44 parts toluene. To this slurry are added 136 parts Alfol 1218 and the mixture is heated to 100° C. To the heated mixture is added a freshly prepared solution of 8 parts methanesulfonic acid in 44 parts Alfol 8-10 followed by heating to 150° C. and reacting at temperature for 5 hours while removing toluene and water of esterification. Esterification at this point is at about 90%. Over 0.25 hour, 14.9 parts butanol are added followed by refluxing until the net acid number is less than 4, indicating 95% esterification. The materials are stripped and filtered.

## EXAMPLE 46-E

The product prepared according to the procedure of Example 27 (2022 parts) is mixed with an additional 80

parts of aromatic hydrocarbon then 744 parts additional aromatic hydrocarbon are added followed by 1756 parts behenyl alcohol. 49.7 parts methanesulfonic acid and an additional 142 parts aromatic hydrocarbon. The batch is heated to 157° C. and is maintained at 157°-160° C. while N<sub>2</sub> blowing until the acid number is below 6. The product is cooled, then collected.

## EXAMPLES OF INCORPORATION OF CARBONYL-AMINO GROUP

The following examples serve to illustrate the preparation of nitrogen-containing esters of the carboxy-containing interpolymers used in this invention and are not intended as limiting thereof. Unless indicated otherwise, all parts and percentages are by weight and temperatures are in degrees Celsius.

## EXAMPLE 1-N

To the esterified interpolymer of Example 1-E is added 20 aminopropyl morpholine (3.71 parts; 10% in excess of the stoichiometric amount required to neutralize the remaining free carboxy radicals) and the resulting mixture is heated to 150°-150° C./10 mm. Hg to distill off toluene and any other volatile components. The stripped product is mixed with an additional amount of mineral oil (12 parts) and filtered. The filtrate is a mineral oil solution of the nitrogen-containing mixed ester having a nitrogen content of 0.16-0.17%.

## EXAMPLE 2-N-12-N

In each of these Examples, the procedure of Example 1-N is followed employing the indicated esterified interpolymer.

| Example | Esterified Interpolymer Example |
|---------|---------------------------------|
| 2-N     | 2-E                             |
| 3-N     | 3-E                             |
| 4-N     | 4-E                             |
| 5-N     | 5-E                             |
| 6-N     | 6-E                             |
| 7-N     | 7-E                             |
| 8-N     | 8-E                             |
| 9-N     | 9-E                             |
| 10-N    | 10-E                            |
| 11-N    | 11-E                            |
| 12-N    | 12-E                            |

## EXAMPLE 13-N

The procedure of Example 1-N is followed except that 50 N-aminoethyl- and 1-methyl-4-aminoethyl piperazine (0.1 mole consumed per carboxy equivalent of the interpolymer) is used in place of aminopropyl morpholine.

## EXAMPLE 14-N

The procedure of Example 1-N is followed except that 55 dimethylamino-ethylamine is substituted for the aminopropyl morpholine used on a molar basis.

## EXAMPLE 15-N

The procedure of Example 1-N is followed except that 60 dibutylamino-propylamine is substituted for the aminopropyl morpholine on a molar basis.

## EXAMPLE 16-N

The procedure of Example 1-N is followed except that 65 the aminopropyl morpholine used is replaced on a chemical equivalent basis with N-aminoethyl pyrrole.

## EXAMPLE 17-N

The procedure of Example 1-N is followed except that the aminopropyl morpholine used is replaced on a chemical equivalent basis with N-aminophenyl oxazolidone.

## EXAMPLE 18-N

The procedure of Example 1-N is followed except that the aminopropyl morpholine used is replaced on a chemical equivalent basis with 1-aminoethyl 2-heptadecylimidazoline.

## EXAMPLE 19-N

The procedure of Example 1-N is followed except that the aminopropyl morpholine used is replaced on a chemical equivalent basis with 4-aminobutyl pyridine.

## EXAMPLE 20-N

Aminopropyl morpholine (35.2 parts) is added to the mixture of Example 15-E, before stripping dropwise over a period of 20 minutes. The mixture is maintained at 150° C. for an additional 30 minutes then cooled with stirring. The mixture is stripped from 50° C. to 141° C. at a pressure of 102 mm. Hg., then permitted to cool. At 100° C., mineral oil (617 parts) is added. Cooling is continued to 60° C. At 60° C., diatomaceous earth (36 parts) is added and the mixture is heated to 100° C. The mixture is maintained at 100°-105° C. for one hour with stirring and then filtered.

## EXAMPLE 21-N

Following substantially the procedure of Example 20-N, 8 parts aminopropyl morpholine are added to an ester prepared according to the procedure of Example 16-E, before stripping.

## EXAMPLE 22-N

The procedure of Example 20-N is repeated with the mixture, before stripping, of Example 17-E.

## EXAMPLE 23-N

Aminopropylmorpholine (15.65 parts) is added dropwise over a period of 10 minutes to the ester of Example 18-E, before stripping. The temperature of the mixture is maintained at 155° C. for 1 hour and then cooled under a nitrogen sweep. Ethyl Antioxidant 733 (1.48 parts) is added to the mixture. The mixture is stripped at 143° C. and 99 mm. Hg. pressure, cooled under nitrogen sweep, then mineral oil is added to provide a total of 63% dilution. Ethyl Antioxidant 733 (1.79 parts) is added and the mixture is stirred for 30 minutes. The mixture is heated to 60° C. while stirring with a nitrogen sweep of 0.5 standard cubic feet per hour. Diatomaceous earth (18 parts) is added to the mixture. The mixture is heated to 90° C. The temperature of the mixture is maintained at 90°-100° C. for 1 hour and then filtered through a pad of 18 parts diatomaceous earth in a heated funnel.

## EXAMPLE 24-N

The procedure of Example 23-N is repeated with the ester, before stripping, of Example 19-E.

## EXAMPLE 25-N

Aminopropyl morpholine (12.91 parts) is added to the mixture of Example 20-E, before stripping. The mixture is

heated under reflux conditions for an additional 4 hours. Diatomaceous earth (30 parts) and a neutral paraffinic oil (302 parts) are added to the mixture which is then stripped. The residue is filtered to yield 497.4 parts of an orange-brown viscous liquid.

## EXAMPLE 26-N

Aminopropyl morpholine (27.91 parts) is added to the mixture of Example 21-E, before stripping, which is then heated under reflux conditions for an additional 5 hours. Diatomaceous earth (60 parts) is added to the mixture which is then stripped, 600 parts of polymer remaining in the vessel. A neutral paraffinic oil (600 parts) is added to the mixture which is then homogenized. The mixture is filtered through a heated funnel to yield 1063 parts of a clear orange-brown viscous liquid.

## EXAMPLE 27-N

20 To an ester prepared as in Example 23-E, before stripping and filtration, is added at 150° C., 6.3 parts aminopropyl morpholine. The materials are heated at 150° C. for 0.5 hour, 2.3 parts alkylated diphenyl amine and 68 parts Cross L-40 oil are added followed by stripping to 150° C. at 40-50 mm Hg. The residue is filtered.

## EXAMPLE 28-N

30 Aminopropyl morpholine (15.6 parts) is added to the mixture of Example 22-E, before stripping, which is then heated under reflux conditions for an additional 5 hours. The mixture is stripped to yield 304 parts of a yellow-orange viscous liquid. Diatomaceous earth (30 parts) and a neutral paraffinic oil (304 parts) are added to the mixture which is then homogenized. The mixture is filtered through a heated funnel to yield 511 parts of a clear amber viscous liquid.

## EXAMPLE 29-N

40 Aminopropyl morpholine (1.3 parts) is added to the mixture of Example 24-E, before stripping, which is then heated for an additional 1 hour at 150° C. The mixture is cooled to 80° C. and 1.84 parts Ethyl Antioxidant 733 is added. The mixture is stripped at 143° C. and 100 mm. Hg, 302 parts mineral oil and 2.18 parts Ethyl Antioxidant 733 are added, and the mixture is stirred while maintaining 90° C. with nitrogen blowing. Diatomaceous earth (44 parts) is added to the mixture which is stirred for 1 hour at 90°-95° C., then filtered to yield 1312 parts of a dark brown clear viscous liquid.

## EXAMPLE 30-N

50 Aminopropylmorpholine (2.33 parts) is added to the mixture of Example 25-E, before stripping, which is heated at 153°-154° C. for 1.3 hour. Ethyl Antioxidant 733 (2.06 parts) is added to the mixture. The mixture is stripped at 142° C. and 100 mm. Hg, 481 parts mineral oil are added, then 2.5 parts Ethyl Antioxidant 733 is added with stirring. Diatomaceous earth (25 parts) is added to the mixture, the temperature is maintained at 70° C. for 45 minutes and then increased to 110° C. The mixture is filtered through 25 parts diatomaceous earth.

## EXAMPLE 31-N

60 65 Aminopropyl morpholine (14.3 parts) is added dropwise over 0.25 hour to the mixture of Example 26-E, before stripping then maintained at 149°-150° C. for 0.5 hour. The

mixture is stripped at 140° C. and 100 mm. Hg, cooled to 50° C., then 338 parts mineral oil and 19 parts diatomaceous earth are added. The temperature is maintained at 100°–105° C. for 1.5 hours and then the materials are filtered through 18 parts additional diatomaceous earth.

#### EXAMPLE 32-N

To an ester prepared as in Example 37-E, but before the final stripping are added 5.8 parts aminopropyl morpholine, followed by heating for 1 hour at 150° C then addition of 1 part alkylated diphenyl amine. The batch is vacuum stripped and filtered.

#### EXAMPLE 33-N

Add 15 parts aminopropylmorpholine and di-tert-butyl phenol (1.04 parts) to the mixture of Example 42-E, before stripping and filtration. Vacuum strip the mixture at 150° C. and 100 mm Hg. Add a second portion of di-tert-butyl phenol (1.04 parts) along with diatomaceous earth (16 parts). Cool the mixture to 100° C. and filter through a hot funnel.

#### EXAMPLE 34-N

Add Ethyl Antioxidant 733 (4.6 parts) and 30 parts aminopropylmorpholine to the product of Example 43-E before stripping and filtration. Vacuum strip the mixture at 150° C. and 20 mm Hg. Cool the mixture to 100° C., add 4.6 parts Ethyl Antioxidant 733 and 36 parts diatomaceous earth, then filter the mixture through a heated funnel.

#### EXAMPLE 35-N

A product prepared as in Example 44-E, before stripping and filtration, is reacted with 7.7 parts of aminopropyl morpholine, mixed for 0.25 hour, then stripped at 150°–160° C. at 25 mm Hg. Alkylated diphenyl amine(1 part) and 88 parts Cross L-40 oil are added and the material is filtered.

#### EXAMPLE 36-N

A product prepared as in Example 45-E before stripping and filtration, is reacted with 6.3 parts of aminopropyl morpholine, mixed for 0.25 hour, stripped at 150°–160° C. at 25 mm Hg. 2.3 parts alkylated diphenyl amine and 88 parts Cross L-40 oil are added and the material is filtered.

As noted above, the present invention is directed to mixtures of esters. The following examples are intended to illustrate compositions of this invention. The compositions are conveniently prepared by simply mixing the esters, usually at temperature ranging between ambient up to the decomposition point of the composition, more often at temperatures ranging from about ambient up to about 100° C.

TABLE 1

| Product of Example | Example |    |    |    |    |    |    |    |   |
|--------------------|---------|----|----|----|----|----|----|----|---|
|                    | (wt %)  | A  | B  | C  | D  | E  | F  | G  | H |
| 27-N               | 50      | 60 | 70 | 80 | 60 |    | 70 |    |   |
| 21-N               | 50      | 40 | 30 | 20 |    | 20 |    |    |   |
| 15-E               |         |    |    |    | 40 |    | 30 | 30 |   |
| 23-E               |         |    |    |    |    | 80 |    | 70 |   |

The mixtures of esterified interpolymers of this invention are useful as viscosity-improving additives for lubricating

oil compositions. As noted above, they provide exceptional pour point depressant properties without an adverse impact on higher temperature viscosity. Nitrogen-containing materials also provide enhanced dispersancy.

5 Lubricating oil compositions of this invention comprise a major amount of an oil of lubricating viscosity and a minor amount of the mixtures of this invention. By a major amount is meant more than 50% by weight. Thus, for example, 51%, 80% and 99% are major amounts. A minor amount is less than 50% by weight. Examples of minor amounts are 1%, 10 20% and 49%.

As noted above, the compositions usually are prepared in a diluent to to facilitate handling.

15 The mixtures of this invention are used in effective amounts to provide the desired pour point and viscosity index. Typically, on a neat chemical basis, the are employed to provide from about 0.01 to about 10% by weight, more often from about 0.20% to about 5% by weight of esterified interpolymers.

#### The Oil of Lubricating Viscosity

The lubricating compositions and methods of this invention employ an oil of lubricating viscosity, including natural and synthetic oils and mixtures thereof.

25 Natural oils include animal oils and vegetable oils (e.g. castor oil, lard oil) as well as mineral lubricating oils such as liquid petroleum oils and solvent-treated, acid treated, and/or hydrotreated mineral lubricating oils of the paraffinic, 30 naphthenic or mixed paraffinic-naphthenic types. Oils of lubricating viscosity derived from coal or shale are also useful. Synthetic lubricating oils include hydrocarbon oils and halosubstituted hydrocarbon oils such as polymerized and interpolymerized olefins, etc. and mixtures thereof, 35 alkylbenzenes, polyphenyl, (e.g., biphenyls, terphenyls, alkylated polyphenyls, etc.), alkylated diphenyl ethers and alkylated diphenyl sulfides and the derivatives, analogs and homologues thereof and the like.

40 Alkylene oxide polymers and interpolymers and derivatives thereof where their terminal hydroxyl groups have been modified by esterification, etherification, etc., constitute another useful class of known synthetic lubricating oils.

Another suitable class of synthetic lubricating oils that can be used comprises the esters of di- and polycarboxylic acids and those made from C<sub>5</sub> to C<sub>20</sub> monocarboxylic acids and polyols and polyolethers.

45 Other synthetic lubricating oils include liquid esters of phosphorus-containing acids, polymeric tetrahydrofurans and the like, silicon-based oils such as the polyalkyl-polyaryl-, polyalkoxy-, or polyaryloxy-siloxane oils and silicate oils.

50 Unrefined, refined and rerefined oils, either natural or synthetic (as well as mixtures of two or more of any of these) 55 of the type disclosed hereinabove can be used in the compositions of the present invention. Unrefined oils are those obtained directly from natural or synthetic sources without further purification treatment. Refined oils are similar to the unrefined oils except they have been further treated in one or more purification steps to improve one or more properties. Rerefined oils are obtained by processes similar to those used to obtain refined oils applied to refined oils which have been already used in service. Such rerefined oils often are additionally processed by techniques directed to removal of 60 spent additives and oil breakdown products.

65 Specific examples of the above-described oils of lubricating viscosity are given in Chambefin, Ill., U.S. Pat. No.

4,326,972 and European Patent Publication 107,282, both of which are hereby incorporated by reference for relevant disclosures contained therein.

A basic, brief description of lubricant base oils appears in an article by D. V. Brock, "Lubrication Engineering", Volume 43, pages 184-5, March, 1987, which article is expressly incorporated by reference for relevant disclosures contained therein.

#### Other Additives

As mentioned, lubricating oil compositions of this invention may contain other components. The use of such additives is optional and the presence thereof in the compositions of this invention will depend on the particular use and level of performance required. Thus the other additive may be included or excluded. The compositions may comprise a zinc salt of a dithiophosphoric acid. Zinc salts of dithiophosphoric acids are often referred to as zinc dithiophosphates, zinc O,O-dihydrocarbyl dithiophosphates, and other commonly used names. They are sometimes referred to by the abbreviation ZDP. One or more zinc salts of dithiophosphoric acids may be present in a minor amount to provide additional extreme pressure, anti-wear and anti-oxidancy performance.

In addition to zinc salts of dithiophosphoric acids discussed hereinabove, other additives that may optionally be used in the lubricating oils of this invention include, for example, detergents, dispersants, viscosity improvers, oxidation inhibiting agents, pour point depressing agents, extreme pressure agents, anti-wear agents, color stabilizers and anti-foam agents. The above-mentioned dispersants and viscosity improvers may be used in addition to the additives of this invention.

Auxiliary extreme pressure agents and corrosion and oxidation inhibiting agents which may be included in the compositions of the invention are exemplified by chlorinated aliphatic hydrocarbons, organic sulfides and polysulfides, phosphorus esters including dihydrocarbon and trihydrocarbon phosphites, molybdenum compounds, and the like.

Other oxidation inhibiting agents include materials such as alkylated diphenyl amines, hindered phenols, especially those having tertiary alkyl groups such as tertiary butyl groups in the position ortho to the phenolic —OH group, and others. Such materials are well known to those of skill in the art.

Auxiliary viscosity improvers (also sometimes referred to as viscosity index improvers or viscosity modifiers) may be included in the compositions of this invention. Viscosity improvers are usually polymers, including polyisobutenes, polymethacrylic acid esters, hydrogenated diene polymers, polyalkyl styrenes, esterified styrene-maleic anhydride copolymers, hydrogenated alkenylarene-conjugated diene copolymers and polyolefins. Multifunctional viscosity improvers, other than those of the present invention, which also have dispersant and/or anti-oxidancy properties are known and may optionally be used in addition to the products of this invention. Such products are described in numerous publications including those mentioned in the Background of the Invention. Each of these publications is hereby expressly incorporated by reference.

Pour point depressants other than those of this invention may be included in the lubricating oils described herein. Those which may be used are described in the literature and are well-known to those skilled in the art; see for example, page 8 of "Lubricant Additives" by C. V. Smalheer and R. Kennedy Smith (Lezius-Hiles Company Publisher,

Cleveland, Ohio, 1967). Pour point depressants useful for the purpose of this invention, techniques for their preparation and their use are described in U.S. Pat. Nos. 2,387,501; 2,015,748; 2,655,479; 1,815,022; 2,191,498; 2,666,748; 5 2,721,877; 2,721,878; and 3,250,715 which are expressly incorporated by reference for their relevant disclosures.

Anti-foam agents used to reduce or prevent the formation of stable foam include silicones or organic polymers. Examples of these and additional anti-foam compositions 10 are described in "Foam Control Agents", by Henry T. Kerner (Noyes Data Corporation, 1976), pages 125-162.

Detergents and dispersants may be of the ash-producing or ashless type. The ash-producing detergents are exemplified by oil soluble neutral and basic salts of alkali or alkaline 15 earth metals with sulfonic acids, carboxylic acids, phenols or organic phosphorus acids characterized by a least one direct carbon-to-phosphorus linkage.

The term "basic salt" is used to designate metal salts 20 wherein the metal is present in stoichiometrically larger amounts than the organic acid radical. Basic salts and techniques for preparing and using them are well known to those skilled in the art and need not be discussed in detail here.

Ashless detergents and dispersants are so-called despite 25 the fact that, depending on its constitution, the detergent or dispersant may upon combustion yield a nonvolatile residue such as boric oxide or phosphorus pentoxide; however, it does not ordinarily contain metal and therefore does not yield a metal-containing ash on combustion. Many types are 30 known in the art, and any of them are suitable for use in the lubricants of this invention. The following are illustrative:

(1) Reaction products of carboxylic acids (or derivatives thereof) containing at least about 34 and preferably at least about 54 carbon atoms with nitrogen containing compounds such as amine, organic hydroxy compounds such as phenols and alcohols, and/or basic inorganic materials. Examples of these "carboxylic dispersants" are described in British Patent number 1,306,529 and in many U.S. patents including the following:

|           |           |           |
|-----------|-----------|-----------|
| 3,163,603 | 3,381,022 | 3,542,680 |
| 3,184,474 | 3,399,141 | 3,567,637 |
| 3,215,707 | 3,415,750 | 3,574,101 |
| 3,219,666 | 3,433,744 | 3,576,743 |
| 3,271,310 | 3,444,170 | 3,630,904 |
| 3,272,746 | 3,448,048 | 3,632,510 |
| 3,281,357 | 3,448,049 | 3,632,511 |
| 3,306,908 | 3,451,933 | 3,697,428 |
| 3,311,558 | 3,454,607 | 3,725,441 |
| 3,316,177 | 3,467,668 | 4,194,886 |
| 3,340,281 | 3,501,405 | 4,234,435 |
| 3,341,542 | 3,522,179 | 4,491,527 |
| 3,346,493 | 3,541,012 | RE 26,433 |
| 3,351,552 | 3,541,678 |           |

(2) Reaction products of relatively high molecular weight aliphatic or alicyclic halides with amines, preferably polyalkylene polyamines. These may be characterized as "amine dispersants" and examples thereof are described for example, in the following U.S. patents:

|           |           |
|-----------|-----------|
| 3,275,554 | 3,454,555 |
| 3,438,757 | 3,565,804 |

(3) Reaction products of alkyl phenols in which the alkyl groups contains at least about 30 carbon atoms with

aldehydes (especially formaldehyde) and amines (especially polyalkylene polyamines), which may be characterized as "Mannich dispersants". The materials described in the following U.S. patents are illustrative:

|           |           |
|-----------|-----------|
| 3,413,347 | 3,725,480 |
| 3,697,574 | 3,726,882 |
| 3,725,277 |           |

(4) Products obtained by post-treating the carboxylic amine or Mannich dispersants with such reagents as urea, thiourea, carbon disulfide, aldehydes, ketones, carboxylic acids, hydrocarbon-substituted succinic anhydrides, nitriles, epoxides, boron compounds, phosphorus compounds or the like. Exemplary materials of this kind are described in the following U.S. patents:

|           |           |           |           |
|-----------|-----------|-----------|-----------|
| 3,036,003 | 3,282,955 | 3,493,520 | 3,639,242 |
| 3,087,936 | 3,312,619 | 3,502,677 | 3,649,229 |
| 3,200,107 | 3,366,569 | 3,513,093 | 3,649,659 |
| 3,216,936 | 3,367,943 | 3,533,945 | 3,658,836 |
| 3,254,025 | 3,373,111 | 3,539,633 | 3,697,574 |
| 3,256,185 | 3,403,102 | 3,573,010 | 3,702,757 |
| 3,278,550 | 3,442,808 | 3,579,450 | 3,703,536 |
| 3,280,234 | 3,455,831 | 3,591,598 | 3,704,308 |
| 3,281,428 | 3,455,832 | 3,600,372 | 3,708,522 |
|           |           |           | 4,234,435 |

(5) Polymers and copolymers of oil-solubilizing monomers such as decyl methacrylate, vinyl decyl ether and high molecular weight olefins with monomers containing polar substituents, e.g., aminoalkyl acrylates or methacrylates, acrylamides and poly-(oxyethylene)-substituted acrylates. These may be characterized as "polymeric dispersants" and examples thereof are disclosed in the following U.S. patents:

|           |           |
|-----------|-----------|
| 3,329,658 | 3,666,730 |
| 3,449,250 | 3,687,849 |
| 3,519,565 | 3,702,300 |

The above-noted patents are incorporated by reference herein for their disclosures of ashless dispersants.

The above-illustrated additives may each be present in lubricating compositions at a concentration of as little as 0.001% by weight, usually ranging from about 0.01% to about 20% by weight. In most instances, they each contribute from about 0.1% to about 10% by weight, more often up to about 5% by weight.

The various additives described herein can be added directly to the lubricant. Preferably, however, they are diluted with a substantially inert, normally liquid organic diluent such as mineral oil, naphtha, benzene, toluene or xylene, to form an additive concentrate. Preferred additive concentrates contain the diluents referred to hereinabove. These concentrates usually comprise from about 0.01 to about 90% by weight, often about 0.1 to about 80% by weight of the compositions of this invention and may contain, in addition, one or more other additives known in the art or described hereinabove. Concentrations such as 15%, 20%, 30% or 50% or higher may be employed.

The lubricating compositions of this invention are illustrated by the examples in the following Table. The lubricating compositions are prepared by combining the specified ingredients, individually or from concentrates, in the indicated amounts and oil of lubricating viscosity to make the

total 100 parts by weight. The amounts shown are parts by weight and, unless indicated otherwise, are amounts of chemical present on an oil-free basis. Thus, for example, an additive comprising 50% oil used at 10% by weight in a blend, provides 5% by weight of chemical. Amounts of components referred to by example number are as prepared. These examples are presented for illustrative purposes only, and are not intended to limit the scope of this invention.

In the Examples of Table 2, the mixtures of esters of Examples A-D of Table 1 are combined in the indicated amounts with a mineral oil of lubricating viscosity, 0.8% of an ethylene-propylene viscosity improver, 1.81% of a polybutene ( $M_n \approx 1300$ ) substituted succinic anhydride-ethylene polyamine reaction product, 0.75% of a mixture of esters of succinimides derived from polybutene ( $M_n \approx 1000$ ) substituted succinic anhydride, 0.6% of di-(nonylphenyl) amine, 0.25% of a sulfurized olefin containing about 19% sulfur, 0.84% of a zinc dialkyl dithiophosphate, 0.31% of a calcium overbased (Metal ratio (MR)  $\approx 3.5$ , 0.15% of calcium overbased (MR  $\approx 20$ ) alkylbenzene sulfonic acid, 0.07% calcium overbased (MR  $\approx 2.8$ ) alkyl benzene sulfonic acid, 0.10% of sodium overbased (% Na  $\approx 25$ ) polybutene ( $M_n \approx 1000$ ) substituted succinic acid, 0.17 T of Mg overbased (MR  $\approx 14$ ) alkylbenzene sulfonic acid and 11 ppm (parts per million parts lubricating oil composition) of a silicone antifoam.

TABLE 2

| Component (wt. %) | Example |     |     |     |     |     |     |
|-------------------|---------|-----|-----|-----|-----|-----|-----|
|                   | I       | II  | III | IV  | V   | VI  | VII |
| A                 | 0.2     | 0.4 |     |     |     |     |     |
| B                 |         |     | 0.2 | 0.4 |     |     |     |
| C                 |         |     |     |     | 0.2 | 0.4 |     |
| D                 |         |     |     |     |     |     | 0.5 |

While the invention has been explained in relation to its preferred embodiments, it is to be understood that various modifications thereof will become apparent to those skilled in the art upon reading the specification. Theretore, it is to be understood that the invention disclosed herein is intended to cover such modifications that fall within the scope of the appended claims.

What is claimed is:

1. A composition comprising a mixture of esterified carboxy-containing interpolymers, said interpolymers having a reduced specific viscosity (RSV) of from about 0.05 to about 2 and being derived from at least two monomers comprising (i) an aliphatic olefin containing from 2 to about 30 carbon atoms or a vinyl aromatic monomer and (ii) an alpha, beta-unsaturated acylating agent, said mixture being characterized by the presence therein of at least two members of the group consisting of

(I) an ester which within its polymeric structure consists essentially of

(A) pendant carboxylic ester groups which are derived from the carboxy groups of said interpolymers, said carboxylic ester groups containing at least 8 carbon atoms;

(II) an ester which is a mixed ester of said carboxy-containing interpolymers and being characterized by the presence within its polymeric structure of at least one of each of two ester groups:

(B) relatively high molecular weight pendant carboxylic ester groups containing at least eight aliphatic carbon atoms, and

(C) relatively low molecular weight pendant carboxylic ester groups containing no more than seven aliphatic

- carbon atoms, wherein the molar ratio of (B):(C) is (70-95):(5-30);
- (III) an ester which is a nitrogen-containing ester, and which within its polymeric structure consists essentially of
- (A) pendant carboxylic ester groups which are derived from the carboxy groups of said interpolymers, said carboxylic ester groups containing at least 8 carbon atoms, and
- (D) pendant carbonyl-amino groups derived from amino compounds having an average of from 1 to about 1.1 primary or secondary amino group, wherein the molar ratio of carboxy groups of said interpolymers esterified to provide (A) to carboxy groups of said interpolymers neutralized to provide (D) is in the range of from about 85:15 to about 99:1; and
- (IV) an ester which is a nitrogen-containing ester, which is a mixed ester of said carboxy-containing interpolymers and being characterized by the presence within its polymeric structure of at least one of each of three groups:
- (B) relatively high molecular weight pendant carboxylic ester groups containing at least eight aliphatic carbon atoms,
- (C) relatively low molecular weight pendant carboxylic ester groups containing no more than seven aliphatic carbon atoms, and
- (E) pendant carbonyl-amino groups derived from amino compounds having an average of from 1 to about 1.1 primary or secondary amino group, wherein the molar ratio of (B):(C):(E) is (60-94):(5-30):(1-15); and wherein the at least two members include at least one ester having the carboxylic ester group (A) and at least one ester having the carboxylic ester groups (B) and (C).
2. The composition of claim 1 wherein the interpolymers have RSV ranging from about 0.08 to about 1.2.
3. The composition according to claim 2 wherein the RSV range from 0.08 to about 0.9.
4. The composition of claim 1 wherein the aliphatic olefin is an alpha olefin.
5. The composition of claim 1 wherein the vinyl aromatic monomer is styrene or a substituted styrene.
6. The composition of claim 1 wherein the alpha,beta-unsaturated acylating agent is an aliphatic carboxylic acid, anhydride, or esters thereof.
7. The composition of claim 1 wherein the alpha, beta-unsaturated acid, anhydride or ester is at least one member selected from the group consisting of maleic acid or anhydride, itaconic acid or anhydride, fumaric acid,  $\alpha$ -methylene glutaric acid, acrylic acid, methacrylic acid or an ester of any of these.
8. The composition of claim 1 wherein the ester groups of (A) have from 8 to about 30 carbon atoms.
9. The composition of claim 8 wherein the ester groups of (A) are selected from the group of ester groups having from 12 to 18 carbon atoms or mixtures of ester groups having from 12 to 18 carbon atoms.
10. The composition of claim 1 wherein the relatively high molecular weight carboxylic ester groups of (B) have from 8 to about 30 carbon atoms and the relatively low molecular weight carboxylic ester groups of (C) have from 3 to 5 carbon atoms.
11. The composition of claim 1 wherein each interpolymers is derived from styrene and maleic anhydride.
12. The composition of claim 11 wherein each interpolymers is further derived from a methacrylic acid ester.
13. The composition of claim 1 wherein the mole ratios of (i):(ii) range from about 1:2 to about 3:1.
14. The composition of claim 1 wherein at least one amino compound is a polyamino compound.
15. The composition of claim 14 wherein the polyamino compound has one primary or secondary amino group and at least one tertiary amino group.
16. The composition of claim 1 wherein the mixture of esters comprises at least one of esters (I) and (II) and at least one of nitrogen-containing esters (III) and (IV).
17. The composition of claim 1 wherein the mixture of esters comprises (I) and (II).
18. The composition of claim 1 wherein the mixture of esters comprises nitrogen-containing esters (III) and (IV).
19. The composition of claim 1 comprising from about 1 to about 99% by weight of esters having carboxylic ester group (A) and from about 99 to about 1% by weight of esters having carboxylic ester groups (B) and (C).
20. The composition of claim 19 comprising from about 1 to about 99% by weight of (I) and from about 99% to about 1% by weight of (II).
21. The composition of claim 19 comprising from about 1 to about 99% by weight of (III) and from about 99% to about 1% by weight of (IV).
22. An additive concentrate composition comprising a substantially inert normally liquid organic diluent and from about 0.01 to about 90% by weight of the composition of claim 1.
23. A lubricating oil composition comprising a major amount of an oil of lubricating viscosity and a minor amount of the composition of claim 1.
24. A lubricating oil composition comprising a major amount of an oil of lubricating viscosity and a minor amount of the composition of claim 22.
25. The additive concentrate of claim 1 further containing a viscosity improver, and optionally, at least one oxidation inhibiting agent.
26. A composition useful as a pour point depressant for hydrocarbon based liquids, prepared by a process comprising mixing together two or more esterified carboxy-containing interpolymers having a reduced specific viscosity of from about 0.05 to about 2, said interpolymers being derived from at least two monomers comprising (i) an aliphatic olefin containing from 2 to about 30 carbon atoms or a vinyl aromatic monomer and (ii) an alpha, beta-unsaturated acylating agent, said mixture being characterized by the presence therein of at least two members of the group consisting of
- (I) an ester which within its polymeric structure consists essentially of
- (A) pendant carboxylic ester groups which are derived from the carboxy groups of said interpolymers, said carboxylic ester groups containing at least 8 carbon atoms;
- (II) an ester which is a mixed ester of said carboxy-containing interpolymers and being characterized by the presence within its polymeric structure of at least one of each of two ester groups:
- (B) relatively high molecular weight pendant carboxylic ester groups containing at least eight aliphatic carbon atoms, and
- (C) relatively low molecular weight pendant carboxylic ester groups containing no more than seven aliphatic carbon atoms, wherein the molar ratio of (B):(C) is (70-95):(5-30);
- (III) an ester which is a nitrogen-containing ester, and which within its polymeric structure consists essentially of

- (A) pendant carboxylic ester groups which are derived from the carboxy groups of said interpolymers, said carboxylic ester groups containing at least 8 carbon atoms, and
- (D) pendant carbonyl-amino groups derived from amino compounds having an average of from 1 to about 1.1 primary or secondary amino group, wherein the molar ratio of carboxy groups of said interpolymers esterified to provide (A) to carboxy groups of said interpolymers neutralized to provide (D) is in the range of from about 85:15 to about 99:1; and
- (IV) an ester which is a nitrogen-containing ester, which is mixed ester of said carboxy-containing interpolymers and being characterized by the presence within its polymeric structure of at least one of each of three groups:

- (B) relatively high molecular weight pendant carboxylic ester groups containing at least eight aliphatic carbon atoms,
- (C) relatively low molecular weight pendant carboxylic ester groups containing no more than seven aliphatic carbon atoms, and
- (E) pendant carbonyl-amino groups derived from amino compounds having an average of from 1 to about 1.1 primary or secondary amino group, wherein the molar ratio of (B):(C):(E) is (60-94):(5-30):(1-15),

and wherein the at least two members include at least one ester having the carboxylic ester group (A) and at least one ester having the carboxylic ester groups (B) and (C).

\* \* \* \* \*